

# United States Patent [19]

Coffield et al.

[11] 3,775,099

[45] Nov. 27, 1973

[54] **METHOD OF WINNING COPPER, NICKEL, AND OTHER METALS**

[75] Inventors: **Thomas H. Coffield**, Orchard Lake; **Kestutis A. Keblys**, Southfield, both of Mich.

[73] Assignee: **Ethyl Corporation**, Richmond, Va.

[22] Filed: **July 17, 1970**

[21] Appl. No.: **55,850**

## Related U.S. Application Data

[60] Continuation-in-part of Ser. No. 717,034, Mar. 28, 1968, abandoned, which is a continuation-in-part of Ser. No. 807,987, Mar. 17, 1969.

[52] U.S. Cl. .... **75/119**, 75/103, 75/108, 75/117, 423/150, 423/143, 423/141

[51] Int. Cl. .... **C22b 3/00**

[58] Field of Search ..... 23/203 C; 75/119, 75/103, 108; 423/141, 143, 150

## References Cited

### UNITED STATES PATENTS

|           |         |                     |          |
|-----------|---------|---------------------|----------|
| 1,686,391 | 10/1928 | Muller et al. ....  | 423/141  |
| 2,822,262 | 2/1958  | Benoit et al. ....  | 75/119 X |
| 2,548,728 | 4/1951  | Kincaid et al. .... | 23/203 C |
| 3,252,753 | 5/1966  | Coffield ....       | 23/360   |
| 2,548,727 | 4/1951  | Kincaid et al. .... | 23/203 C |
| 2,952,517 | 9/1960  | Podall et al. ....  | 23/203 C |

### FOREIGN PATENTS OR APPLICATIONS

|         |        |                |          |
|---------|--------|----------------|----------|
| 240,119 | 9/1960 | Australia..... | 23/203 C |
| 583,571 | 9/1959 | Canada .....   | 23/203 C |

|         |        |                     |          |
|---------|--------|---------------------|----------|
| 615,822 | 3/1961 | Canada .....        | 23/203C  |
| 706,316 | 3/1965 | Canada .....        | 23/203 C |
| 323,332 | 1/1930 | Great Britain ..... | 23/203 C |

## OTHER PUBLICATIONS

Blanchard, "Chemical Reviews," Vol. 21, 1937, pp. 3, 10-12.

Primary Examiner—Herbert T. Carter  
Attorney—Donald L. Johnson

[57]

## ABSTRACT

The invention is a process for winning nickel by treating an aqueous ammonium salt solution of nickel salts with a carbon monoxide-containing gas under reducing conditions to produce nickel carbonyl and subsequently recovering nickel therefrom. Optionally, the production of nickel carbonyl can be catalyzed, for example, by cyanide. Also, an essentially water-immiscible solvent for nickel carbonyl can optionally be employed. The aqueous ammoniacal solution is typically an aqueous ammoniacal ammonium chloride, carbonate, sulfate, hydroxide, or mixture thereof. The valuable metals associated with nickel, e.g., copper, cobalt, iron, and precious metals, are also separated and recovered by this process. The general nature of the process allows a wide variety of primary and secondary sources of nickel to be utilized by combining this process with a number of known ore-treatment steps.

24 Claims, 9 Drawing Figures

PATENTED NOV 27 1973

3,775,099

SHEET 1 OF 9



FIGURE 1

INVENTORS

T. H. COFFIELD  
K. KELBLYS



FIGURE 2

INVENTORS

T. H. COFFIELD

K. KEBLYS

PATENTED NOV 27 1973

3,775,099

SHEET 3 OF 9

A



B



FIGURE 3

INVENTORS

T. H. COFFIELD

K. KEBLYS

PATENTED NOV 27 1973

3,775,099

SHEET 4 OF 9



## FIGURE 4

## INVENTORS

T. H. COFFIELD

K. KEBLYS



FIGURE 5

INVENTORS

T. H. COFFIELD

K. KEBLYS

A



B



FIGURE 6

INVENTORS

T. H. COFFIELD  
K. KEBLYS

PATENTED NOV 27 1973

3,775,099

SHEET 7 OF 9



## FIGURE 7

INVENTORS  
T. H. COFFIELD  
K. KEBIYS



FIGURE 8

INVENTORS

T. H. COFFIELD

K. KEBLEYS

PATENTED NOV 27 1973

3,775,099

SHEET 9 OF 9



FIGURE 9

INVENTORS  
T. H. COFFIELD  
K. KEBLYS

## METHOD OF WINNING COPPER, NICKEL, AND OTHER METALS

This application is a continuation-in-part of applications Ser. No. 717,034, filed Mar. 28, 1968 and now abandoned, and Ser. No. 807,987, filed Mar. 17, 1969.

### BACKGROUND OF THE INVENTION

Winning metals has been a human activity since time immemorial. Civilization has grown with this art; and it is safe to say that the production of metals is the genesis and sustenance of many aspects of modern technology. At the present time, mankind utilizes metals at a large and rapidly increasing rate. For this reason, improvements in techniques for obtaining metals have immediate interest.

The above facts are adequately illustrated by the history of copper. Mankind emerged from the Stone Age upon discovery of copper in its native form. The dawn of the Bronze Age was circa 8,000 B.C. — when it was discovered that this copper-tin alloy could be readily shaped into implements and weapons. Copper deposits on Cyprus were worked as early as 3,000 B.C. by the Egyptians and these deposits became the chief source of the metal for the Roman Empire. In 1556, Agricola recorded the history of copper. In 1963, world refined copper output exceeded 3,800,000 short tons.

Nickel was isolated by Cronstedt in 1751. By 1804, the properties of the pure metal were known with reasonable accuracy.

Referring to the section on copper in Kirk-Othmer *Encyclopedia of Chemical Technology*, second edition, volume 6, page 131, and *The Winning of Nickel*, by Boldt, Jr., et al, D. Van Nostrand Co., New York, N. Y. (1967), the production of copper and nickel from ores are tedious, complex processes. Clearly, commerce could not bear the cost of such multi-step processes if these metals were not so important. A detailed discussion of all ramifications of art-known methods for the production of copper and nickel would be out of place here. It is sufficient to relate the following facts.

Copper and nickel are both present in some ores worked today. Since 1899 nickel has been refined by the Mond process which comprises reacting nickel with carbon monoxide to form nickel carbonyl and subsequent decomposition of this product to carbon monoxide and nickel. In the section on nickel in Kirk-Othmer (supra), second edition, volume 13, page 735, (739) there is described a hydrometallurgical refining process for nickel (practiced by Sherritt Gordon Mines Limited of Toronto, Canada). In this process, concentrates of pentlandite,  $(\text{Ni}, \text{Fe})_9\text{S}_8$ , are dissolved in an aerated ammoniacal solution. The nickel, copper and cobalt sulfides dissolve as ammines, with iron remaining in the residue as hydrated ferric oxide. Subsequently, copper is precipitated, and the remaining nickel solution is oxidized to destroy sulfamate. The resultant solution is treated with hydrogen at 35 atmospheres and 190°C. to yield 99.9 percent nickel which is sintered into briquettes.

The Sherritt Gordon process is described in more detail in Boldt, Jr. (supra), page 299 ff. As described therein, the copper is removed from the ammoniacal solution by boiling off ammonia to precipitate cupric sulfide. The last traces of copper are removed by adding  $\text{H}_2\text{S}$ . This must be done before nickel is precipitated

with hydrogen, to avoid contamination of the nickel with copper.

In general, nickel and associated metals are recovered and separated by pyrometallurgical, hydrometallurgical, or electrolytic refining techniques. For sulfide ores, the general operations of roasting, smelting, and converting produce a nickel matte product which is suitable for refining to pure metal electrolytically. In contrast to sulfide ore processing, the oxide ores may be more economically processed by hydrometallurgical or carbonyl processes to produce very high purity nickel. However, this is not true in all cases since one commercial operation utilizes pyrometallurgical techniques to prepare ferronickel from a laterite ore. A roasting operation decreases the sulfur content of a sulfide ore concentrate by about one-half. Previous processes have used multiple hearth furnaces, sintering machines, or fluidized bed reactors. When followed by smelting operations using shaft furnaces, reverberatory furnaces or electric arc furnaces to slag off siliceous and other oxide compounds, a typical nickel sulfide matte containing about 15 percent nickel-copper, 50 percent iron, and 25 percent sulfur is produced. This nickel-sulfide matte is then charged to a converter and air is blown through the charge to oxidize iron sulfide selectively. Usually, horizontal converters are used. Recently a process using a top-blown rotary converter in which an oxygen lance is blown onto the surface of the molten charge has been placed in successful commercial operation. The nickel sulfide matte essentially free of iron produced in the converting operation, typically contains about 48 percent nickel, 27 percent copper, 22 percent sulfur, and less than 1 percent iron. This matte is sulfur deficient and, therefore, contains a metallic phase which must be processed to separate the nickel sulfide and copper sulfide. In one process, a slow cooling step is used whereby the sulfur deficient matte cast from the converter is cooled slowly over a period of several days. The nickel sulfide, copper sulfide, and copper-nickel metallics separate, allowing regular ore dressing operations to be used to separate the solidified matte into its components. Thus, the nickel-copper alloy is removed magnetically and the nickel and copper sulfides are then separated by flotation. The nickel sulfide can then be either sintered to provide 90 percent nickel for direct use by steel producers, or roasted to the oxide, smelted and cast into anodes for electrolytic refining. Alternatively, the nickel sulfide matte can be cast directly into anodes for electro-refining.

In electrolytic refining, metallic nickel of high purity is produced. A major portion of the world's nickel production includes this process as a last step in winning nickel. In addition, the recovery of precious metals and other elements such as cobalt is practiced. A divided electrolytic cell with a porous diaphragm separating the anode and cathode is used in the electrolytic process. The diaphragm prevents impure anolyte from directly contacting the nickel cathode starting sheet. The impure anolyte obtained by solution of the anode is pumped away from the cell to another area where impurities are removed. The nickel cathodes containing 99.9+ percent nickel are removed after about 10 days operation of the cell.

In addition to the Sherritt Gordon process described above, other hydrometallurgical refining processes are commercially employed to win nickel by gaseous reduction of nickel salt solutions derived from both sul-

fide and oxide ores. Preparatory ore-dressing treatments provide a uniform feed for the reduction and leaching process. Leaching procedures vary depending on the particular ore treated. However, the nickel carbonates produced from the aqueous solution are calcined to marketable nickel oxide, or further sintered to upgrade the nickel metal content to about 88 percent. A process to recover nickel and cobalt from a limonitic-type laterite ore from Cuba treated the ore with sulfuric acid at elevated temperature and pressure to dissolve nickel and cobalt preferentially. The iron remained essentially undissolved. The liquid separated from the residue contained 95 percent of the nickel found in the ore. After further purification of the aqueous phase, the nickel sulfate is reacted with hydrogen at high pressure and at about 190°C. to recover most of the nickel as a 99.8 percent pure product.

Nickel is also produced in the form of ferronickel and nickel rondelles. Ferronickel is produced by a pyrometallurgical process of melting, reduction, and refining. One commercial process in New Caledonia reduces the ore with coke in electric furnaces. Another commercial process in Oregon involves mixing molten ore with ferrosilicon and crude ferronickel. By pouring the molten materials back and forth in special ladles, the molten ore is reduced and the resulting ferronickel product contains about 48 percent nickel. This crude product is further refined to lower the impurity level. Nickel rondelles are produced by reacting the ore with coke and gypsum in blast furnaces, blowing the nickel-iron matte and a siliceous flux with air and converting to produce a low-sulfur nickel matte, roasting to the oxide, grinding, compacting, and reducing to the metal with charcoal. The resulting nickel rondelles contain 99 percent nickel.

Data on the reduction of copper (II) salts with carbon monoxide has been published; Byerley et al., *Met. Soc. Conf.*, 24, 183 (1963); *Chem. Abs.* 64, 13441 h (1966). Conversion of aqueous nickel to nickel carbonyl has been disclosed in *Chem. Abs.* 53, 12606 h (1959).

#### SUMMARY OF THE INVENTION

Discoveries on which this invention is based are as follows:

1. The reduction of copper (II) salts to copper metal with carbon monoxide is promoted by the presence of nickel carbonyl, manganese carbonyl, or cobalt carbonyl.
2. With ammoniacal solutions of copper and nickel salts, it is not necessary to separate copper before winning the nickel.
3. Cupric salts can be reduced to copper metal simultaneously and in the same reaction zone wherein nickel carbonyl is produced from nickel (II) salts, via use of carbon monoxide or synthesis gas treatment.
4. The reduction of nickel (II) salts to nickel carbonyl with carbon monoxide is promoted in the presence of a ligand selected from cyanide, sulfide, cysteine, and tartrate.
5. Practically complete conversion and separation of nickel, copper, and cobalt is possible by treating ammonium salt solutions of those metals prepared from an ore, an ore concentrate such as a beneficiated raw ore concentrate, a nickel-iron or a nickel-sulfur matte, or a ferronickel product, with carbon monoxide or synthesis gas under conditions whereby the nickel and cobalt

values are reduced to form metal carbonyl compounds, and the copper is reduced to metallic copper.

Based on these discoveries, this invention is a process for winning nickel by treating a nickel-containing solution of various metal ions with a carbon monoxide-containing gas and forming a nickel carbonyl compound which can be easily separated from the solution and from other metal compounds or metals. Moreover, valuable metals associated with nickel, e.g., cobalt and copper, may be simultaneously converted to carbonyl compounds or reduced to the metallic state and, thereafter, be easily separated and recovered.

In part, this invention also resides in new improved processes for separation of nickel, cobalt, copper, and iron from ores (or other materials) containing these metals. Such processes are outlined below as follows.

A source of nickel, copper, cobalt, and iron, such as a sulfide-type nickel ore concentrate, is treated with aqueous ammonia and aerated. The resulting aqueous ammonia solution — after removal of the precipitated iron — contains nickel, copper and cobalt values as ammine sulfates. This solution is put in a reaction zone having a surface suitable for subsequent copper deposition or alternatively, the solution can be seeded with finely divided copper. In either event, the ammoniacal solution is thereafter treated with carbon monoxide or synthesis gas under pressure. As reduction proceeds, nickel ion is reacted to nickel carbonyl. This can be removed and decomposed thermally to nickel powder. During the reduction step, copper ion is reduced to the metal and deposited. The copper is removed from the reaction zone. During the reduction step, cobalt ion is reduced to the cobalt tetracarbonyl anion which remains in the solution. As such, it can be separated from nickel and copper. The cobalt can be recovered by injecting an oxygen-containing gas into the solution whereby cobalt is oxidized to hydrated cobalt oxide. It is then filtered from the solution and heated to remove the waters of hydration. After cobalt removal, the solution contains ammonium sulfate, which is isolated as a by-product.

Another process for winning nickel is to prepare an ammonium salt solution of a laterite ore by crushing and grinding the ore to a fine uniform feed of approximately constant composition, roasting the ore in a reducing atmosphere typically with producer gas, cooling the reduced ore under non-oxidizing conditions, leaching the reduced ore with an aqueous ammonium salt to solubilize nickel and cobalt. The ammonium salt solution is treated with carbon monoxide under conditions to form nickel and cobalt carbonyl compounds, each of which may be separated and recovered.

Still another process contemplated by this invention is the oxidative leach and carbon monoxide or synthesis gas treatment of a ferronickel product produced from either an oxide or sulfide ore. Recovery of nickel and cobalt proceeds as before from the carbonyl compounds produced.

A still further process for winning nickel is the oxidative leach and reductive carbonylation of a furnace or converter matte produced by conventional procedures from a convenient source of either sulfide or laterite ores. After the matte is produced, it is treated by an oxidative leach with an ammonium salt solution to dissolve the desired metals. Treatment of the resultant solution with a carbon monoxide-containing gas reacts nickel and cobalt, and if present, copper, to the above-

stated forms which can be separated and recovered from the solution.

In addition, nickel may be recovered from scrap metal containing a recoverable quantity of nickel by comminuting the scrap, dissolving the nickel values selectively, using an oxidative leach with an ammonium salt solution and treating said solution with a carbon monoxide-containing gas. The nickel is reduced to a carbonyl compound and separated and recovered from the solution. Other metal values such as copper and cobalt associated with the scrap metal may also be recovered according to this process.

Nickel may also be recovered from manganese nodules found on the deep sea floor. The nodules are comminuted, subjected to a reducing roast, cooled under non-oxidizing conditions, and leached with an aqueous ammonium salt to solubilize the nickel values, as well as copper and cobalt. The solution is treated with a carbon monoxide-containing gas under conditions to form metal carbonyl compounds or the metal itself in the case of copper. The valuable metals are then recovered as previously described.

In each case, briefly described above, a promoter may be employed to accelerate the formation of the carbonyl compounds.

#### DESCRIPTION OF THE DRAWINGS

FIG. 1 is a schematic representation of the production of nickel carbonyl from a solution containing nickel ions by reacting said solution with a carbon monoxide-containing gas in the presence of a catalyst.

FIG. 2 shows in Part A a schematic representation of the Nicaro process for producing a nickel oxide product from ore by a process of drying, reducing and cooling under non-oxidizing conditions, leaching the reduced ore, stripping ammonia from the leach solution, separating nickel carbonate from the solution, and sintering to produce nickel oxide. Part B of FIG. 2 represents the combination of a Nicaro process with reductive carbonylation wherein the schematic representation shows a reductive carbonylation step after the oxidative leach with subsequent metal recovery.

FIG. 3 shows in Part A the preparation of ferronickel from a nickel ore by smelting the ore, desulfurizing the molten ore with sodium carbonate, blowing the desulfurized melt with oxygen to produce a ferronickel product. Part B shows the combination of the smelting operation with an oxidative leach and reductive carbonylation and recovery of nickel metal instead of the ferronickel product.

FIG. 4 is a schematic representation in Part A of the production of nickel rondelles from a nickel sulfide matte. In this process after a laterite ore is sintered and smelted in a blast furnace, the blast furnace matte is converted to a nickel sulfide matte by blowing with air. The converter matte is then roasted in a two-stage process to nickel oxide briquets which are then reduced to nickel rondelles. Part B shows a schematic representation of a process combining the nickel sulfide matte process with an oxidative leach solution and reductive carbonylation to produce nickel metal.

FIG. 5 is a schematic representation in Part A of the Sherritt Gordon process for obtaining nickel briquets from a sulfide ore using a hydrometallurgical process. Part A shows the beneficiation of a sulfide ore and oxidative leach of the nickel concentrate produced with subsequent copper removal and oxydrolisis of the

nickel to nickel sulfate. Reduction of this solution with hydrogen produces a nickel powder which is dried and briquetted. Part B of FIG. 5 represents the combination of the Sherritt Gordon process with reductive carbonylation wherein reductive carbonylation is carried out on the leach solution and nickel metal is recovered.

FIG. 6 is a schematic representation in Part A of the production of nickel by a process of flash smelting a nickel concentrate, converting the molten metals to a nickel sulfide matte, leaching the matte in a two-stage process to separate nickel from copper, reacting the leach solution with black nickel hydroxide to precipitate cobalt, and electrolysis of the nickel-containing solution to produce highly pure nickel cathode sheets. Part B of FIG. 6 schematically represents the combination with reductive carbonylation of the above process wherein an oxidative leach step is carried out after either the flash smelting operation or the converting operation. The leach solution is carbonylated and nickel metal recovered.

FIG. 7 represents in Part A a schematic process for production of nickel from a sulfide ore by a process of converting a nickel concentrate in a top-blown rotary converter to produce a molten nickel sulfide melt which is drastically quenched in water. The granulated melt is subjected to carbonylation under high pressure, and the carbonyls are separated to produce nickel metal and ferronickel. The solid residues from pressure carbonylation are leached and purified to produce other metals. Part B of FIG. 7 shows the combination of reductive carbonylation with the top-blown rotary converter operation described above. After converting a nickel concentrate to a low-sulfur molten nickel matte and quenching, the granulated nickel matte is oxidatively leached and subjected to reductive carbonylation. Nickel metal is recovered.

FIG. 8 is a schematic representation in Part A of a process for winning nickel by roasting a nickel concentrate, smelting the roasted concentrate, and converting the matte produced to a nickel sulfide matte. The nickel sulfide matte is allowed to cool slowly and separates into its various metallic phases. The solid matte is again beneficiated, roasted, and smelted, and the high nickel matte is cast into anodes for electro-winning of nickel metal. In Part B, the combination of oxidative leach and the reductive carbonylation is added after the nickel is roasted, smelted and converted to produce a nickel matte. The matte is leached and carbonylated to produce nickel metal.

FIG. 9 is a schematic representation of a process for recovery of nickel metal from scrap metal. The scrap is comminuted and then oxidatively leached, subjected to reductive carbonylation, and nickel metal is recovered.

#### DESCRIPTION OF PREFERRED EMBODIMENTS

The invention is a process for recovery and separation of nickel and metal values associated therewith derived from a sulfide or laterite source of nickel ore. The process comprises establishing a solution or slurry containing nickel and the metal values associated therewith from which iron has been removed and contacting said solution or slurry with a carbon monoxide-containing gas to form carbonyl compounds of the metal values. The nature and properties of the carbonyl compounds allow easy and complete separation of the metal carbonyl compounds from the solution or slurry.

As a convenient source of metals for the process of this invention, materials rich in nickel such as sulfide or laterite ores and the processed materials derived therefrom such as concentrates, mattes, and leach solutions, and scrap metal, and ocean nodules may be treated. The treatment of the source of nickel and metals associated therewith is largely a matter of choice, depending upon the type of ore, its situation in the natural state, or the economics of obtaining a convenient source of metal values to be treated by the process of this invention.

Establishment of a solution or slurry from the source of ores described above can be by solubilization, selective leaching, or physical separation of metallic constituents, as for example by flotation. In short, any art-recognized method of obtaining a solution or slurry of nickel and associated metals may be used to prepare a solution or slurry suitable for subsequent carbonylation. The concentration of metals in the solution or slurry may vary widely. Indeed, any concentration conveniently obtained may be used to produce nickel and associated metals by the process of this invention. Diluted solutions, saturated solutions, or super-saturated solutions, for example slurries, may be used in the separation and recovery of nickel and associated metals in this process.

Any means which the art has recognized as sufficient to dissolve nickel and its associated metals may be used to prepare a solution or slurry of said nickel and associated metals. The only requirement is that the nickel be in a form that has at least some water-solubility or that it is rendered soluble by the action of a coordinating agent such as ammonia. The anion associated with the nickel is not critical. For example, the nickel may be in the form of the water soluble nickel salts such as nickel acetate, nickel ammonium chloride, nickel ammonium sulfate, nickel bromide, nickel chloride, nickel fluoride, nickel iodide, or nickel sulfate. The nickel may be in a normally insoluble form which is rendered at least partially soluble by an agent such as ammonia. These nickel compounds would include nickel carbonate, basic nickel carbonate, nickel oxide, nickel phosphate, nickel hydroxide, and the like.

The aqueous reaction media may be water or water-containing an ammonium salt. The function of the ammonium salt is to at least partially solubilize the nickel compound. Useful ammonium salts include ammonium chloride, ammonium carbonate, ammonium sulfate, ammonium phosphate, ammonium bromide, ammonium iodide, ammonium phosphite, ammonium sulfite, ammonium cyanide, ammonium fluoride, ammonium sulfide, and the like, including mixtures thereof. The reaction media may also be aqueous ammonium hydroxide.

The concentration of the ammonium salt solution is not critical. As stated above, it is not even required when the nickel compound has some water solubility. When required, a preferred concentration range is from about 0.1 wt. % up to a saturated ammonium salt solution. In general, good results are obtained using a 2-20 wt.% aqueous ammonium salt solution. A most preferred range is from about 3-10 wt. % ammonium salt.

Most preferred aqueous reaction media are ammoniacal ammonium salt solutions. These are solutions of ammonium salts such as the above containing dissolved ammonia. The amount of excess ammonia can range up

to complete saturation of the aqueous media. A preferred amount of ammonia is from about 1-40 wt. % NH<sub>3</sub>. A more preferred range is from 2-20 wt.% NH<sub>3</sub>, and a most preferred NH<sub>3</sub> concentration is from about 2-10 wt.%.

The amount of ammonium salt in the aqueous reaction media should be at least sufficient to provide on an equivalent basis an amount of anions equal to the amount of metallic nickel, copper, or cobalt present.

10 Preferably, the amount of anions provided by the ammonium salt should be in excess of the equivalents of metallic nickel, copper, or cobalt present. A useful range based on the equivalent of nickel, copper, and cobalt present is from stoichiometric to about 100 equivalents of anion per equivalent of the above metals. It is apparent from the above, for example, that a low sulfur matte will require more ammonium salt in the aqueous reaction media than a high sulfur matte because it will contain more metal in the metallic state requiring more anions to be supplied by the ammonium salt to dissolve or leach the matte into solution.

When the nickel is at least partially dissolved, the resultant solution or slurry is treated with a carbon monoxide-containing gas. An amount of the carbon monoxide-containing gas at least sufficient to combine with nickel and its associated metals is introduced into the solution by a wide variety of methods. The particular method of introduction is not critical. The only requirement being that intimate contact of the solution and carbon monoxide-containing gas is established. A preferred carbon monoxide-containing gas is carbon monoxide. However, synthesis gas, a combination of hydrogen and carbon monoxide, may also be used. A preferred method of treating the solution is to introduce the carbon monoxide-containing gas under super-atmospheric pressure. Pressures of carbon monoxide from 50 to about 3,000 psig, may be employed. A preferred range of carbon monoxide pressure is from 50 to about 1,800 psig.

25 40 One skilled in the art will readily see that pressure is not an entirely independent variable but depends upon the system being treated. That is, the type of ore and the type of salt solution will affect the pressure required to carry out efficient carbonylation.

45 Temperatures at which the carbonylation process is carried out are those which facilitate a desirable rate of reaction and also allow convenient processing equipment to be utilized. Temperatures depend on the type of feed and the aqueous reaction media used in the carbonylation process. Thus, the temperature is in many instances dependent upon the pressure, feed and rate of reaction desired. A general range of temperatures under which carbonylation can be carried out are from 50° to about 250°C. A preferred range of temperatures is from about 100° to about 175°C.

50 55 60 65 It has been found that the reaction of the carbon monoxide-containing ammoniacal salt solution is accelerated in the presence of certain promoters. The method by which such acceleration takes place is not fully understood. However, the rate of carbonylation is markedly increased by addition of certain promoters. It has been found that such promoters are ligands selected from alkoxide anions, organic acid anions, inorganic acid anions, and inorganic anions. A preferred group of ligands found to be useful in promoting the carbonylation process are cysteine and tartrate, sulfide and cyanide. A preferred promoter ligand is cyanide

ion. The manner of introducing the promoter into the reaction medium is not critical and the only requirement is that the catalytic species be soluble in the reaction medium. A preferred amount of the promoter or catalyst ligand is a catalyst-to-nickel ratio of 0.01-1 mole of promoter per mole of nickel. A preferred range is from 0.01-0.5. It should be understood that the particular catalyst concentration useful in the process of this invention depends on the reaction system employed and the feed material being carbonylated.

The duration of the reaction is a function of the system being carbonylated and may vary depending on the pressure, temperature, the type of feed, and the solubilizing agent and the use of a catalyst. Under the broad range of conditions employed, carbonylation reaction times of up to about ten hours have been noted. However, under preferred conditions, the reaction is essentially completed after about two hours. In fact, the major portion of the reaction is completed within the first one-half hour when a catalyst is employed. Completion of the reaction is shown by a sharp decrease in rate of pressure drop in the reaction vessel. It should be understood that the reaction time is not a completely independent variable and can be varied according to reasonable requirements of the individual reaction system.

In a preferred process, the nickel and associated metals, after being taken into solution, are carbonylated in an ammonium salt solution. A most preferred embodiment is the use of an aqueous ammoniacal ammonium carbonate solution wherein ammonia and carbon dioxide are added to an aqueous media which is used to leach the nickel and associated metals from their source material. In general, the solutions use a ratio of ammonia-to-metal in the ammonium salt solution of from zero to 1 to about 100 to 1 moles of ammonia per mole of metal. A preferred amount of ammonia in such a system is from 0 to 50 moles of ammonia per mole of metal in the solution. A most preferred range is from 0 to 10 moles of ammonia per mole of metal in solution.

The nickel carbonyl formed by the reaction of the carbon monoxide-containing gas and the nickel may be separated from the reaction solution by taking it up in a water-immiscible, substantially inert solvent for nickel carbonyl or by sweeping out the reaction vessel with additional carbon monoxide-containing gas. The exact nature of the solvent is not critical so long as it is immiscible with water, dissolves nickel carbonyl, and is substantially inert under the reaction conditions. In a preferred embodiment, a solvent less dense than water is used. Nickel carbonyl is soluble in many organic solvents such as paraffins, mixtures thereof, benzene, toluene, and carbon tetrachloride. Preferred solvents are paraffin fractions such as ligroin, gasoline, kerosene, and paraffinic materials such as cyclohexane, heptane, octane, nonane, and the like. Normal or branched chain paraffins can be used as well as mixtures thereof. A most preferred solvent is a saturated aliphatic hydrocarbon such as hexane, heptane, octane, nonane, decane, dodecane, their branched chain derivatives, mixtures of these, and the like.

The amount of solvent which is used is not critical. It is only necessary to use the amount of solvent required to dissolve the desired amount of nickel carbonyl. There is no real upper limit on the amount of organic solvent, this being defined by such considerations

as economics, size of the reaction vessel, ease of separation of nickel carbonyl therefrom, and the like. Generally from 0.1 to 2 volumes of organic solvent are used per unit volume of aqueous reaction media. Preferably from 0.1 to 0.5 volumes are employed.

As stated above, the nickel carbonyl may also be separated from the reaction media by passing a carbon monoxide-containing gas through the solution, allowing the nickel carbonyl to vaporize into the carbon monoxide-containing gas. When the reaction is completed, nickel carbonyl is present both in the vapor phase above the reaction solution and dissolved in the solution itself. As the pressure is released, the vapor phase containing the carbon monoxide-containing gas and vaporized nickel carbonyls is vented to a nickel carbonyl recovery zone, for example, a thermal decomposition zone. Additional carbon monoxide-containing gas is introduced through the solution and nickel carbonyl vaporizes into the gas and it is passed out of the reaction vessel into the recovery zone. Thus, substantially complete removal of nickel carbonyl is obtained. The carbon monoxide-containing gas used to sweep out the nickel carbonyl may be the same as that employed to react with the nickel. As stated above, preferred carbon monoxide-containing gases are carbon monoxide and synthesis gas. The amount of sweep gas is not critical and depends on the reactor size, temperature, and pressure of the system. Generally, from about 1 to 1,000 volumes of the carbon monoxide-containing gas is sufficient.

Referring again to the drawings, FIG. 1 is a schematic representation of the general process of this invention. The block labeled "reductive carbonylation" represents a suitable reactor in which the process is carried out. Any convenient reaction vessel may be utilized within the limitation of sound engineering and economic principles. A feed of aqueous ammine solution containing metal ions; e.g., nickel, copper, cobalt, and the like, is charged to the reactor. Catalyst (e.g., cyanide ion) is added and the reactor is pressurized with a carbon monoxide-containing gas. Any recycle stream containing recovered metal ions from the solution or residue, if any, or additional ammine solution required to adjust the concentration of the reaction solution may be added. The reactor is brought to reaction temperature and the solution agitated mechanically. The beginning of the reaction is signalled by a decrease in the pressure of the carbon monoxide-containing gas. Completion of the reaction is shown by cessation of pressure drop. The nickel carbonyl is then separated from the solution and sent to recovery units. The solution containing cobalt carbonyl compounds is also sent to recover the metals therefrom. Any copper metal present will be deposited in the reactor and can then be recovered. If other impurities in the solution are present, a residue may form and the copper must be separated therefrom.

This general process can be varied as appreciated by one skilled in the art, without departing from the scope of the invention. For example, as described above, a solvent for nickel carbonyl may also be added to the reaction mixture. Its purpose is to selectively solvate the nickel carbonyl formed and provide a means for removing it from the system. The reaction may also be run on a continuous basis with appropriate modifications for maintaining the pressure, temperature and reaction rate. In such a case, the reaction solution with-

drawn must be processed to remove unreacted metal ions and recycle them to the reactor if required.

The process is further illustrated by the following examples. All parts are by weight unless otherwise stated.

#### EXAMPLE 1

A glass lined rocking autoclave was charged with 5.0 g. of copper sulfate pentahydrate, 5.25 g. of nickel sulfate hexahydrate, 21 ml. of concentrated ammonia, 25 ml. of water, and 10 ml. of heptane. The autoclave was pressured with 640 psig. hydrogen and 1,200 psig. carbon monoxide, then heated 2 hours at 150°C.

The resultant mixture consisted of a colorless heptane phase, metallic copper, and a light blue aqueous solution. The heptane phase was siphoned off and combined with subsequent heptane extracts of aqueous phase. The nickel carbonyl and heptane solution was treated with excess bromine in carbon tetrachloride. The resulting mixture was filtered, washed with carbon tetrachloride and dried. This gave 2.55 g. of nickel bromide. This corresponds to a 58 percent yield of nickel carbonyl based on starting nickel sulfate.

The copper metal was filtered, washed and dried in vacuo, yielding 0.90 g. of copper metal. This corresponds to a 71 percent yield based on starting copper sulfate.

This example illustrates that cupric salts present in an ammoniacal aqueous solution can form metallic copper in the presence of hydrogen and carbon monoxide even though nickel salts are present in the pregnant solution. It also illustrates that nickel (II) and salts in aqueous ammoniacal solution form nickel carbonyl in the presence of copper ammines. There is another facet to the example. Specifically, the copper metal and nickel carbonyl were separable in the absence of an overt contamination of either product; even though hydrogen gas was present in the reducing atmosphere. This example also illustrates that it is possible to extract nickel carbonyl with an essentially water-immiscible solution while reductions are taking place.

#### EXAMPLE 2

A pregnant aqueous solution contains in grams per liter:

nickel — 45  
cobalt — 0.7  
copper — 7  
ammonium sulfate — 150  
free ammonia — 95

This solution is treated with 0.05 gram per liter of copper powder (finely divided) and then fed into a pressure vessel. The reaction vessel is charged with heptane so that the ratio of volume of pregnant solution to heptane is 10 to 1.

The pressure vessel is equipped with a stirrer which is activated. Then, the sealed vessel is charged with 800 psig. of synthesis gas at 175°C. The vessel contents are maintained at this temperature for 2 hours. After that time, the stirrer is turned off and the vessel contents allowed to cool to ambient temperature.

Thereafter, the aqueous layer is drawn off and the copper metal removed by filtration. The filtrate is sent downstream for recovery of cobalt values and ammonium sulfate by-products.

The heptane layer is drawn off and the nickel carbonyl separated by distillation. In this example, nine-tenths of the nickel carbonyl is decomposed to form

nickel metal powder. The remaining one-tenth is reacted with bromine to form nickel bromide.

This nickel bromide is used to form nickelocene according to U.S. Pat No. 2,680,758. The nickelocene 5 can be further reacted according to procedures in U.S. Pat. No. 3,054,815, to form other organo nickel compounds. In addition, it is appreciated by a skilled practitioner that nickel carbonyl, nickel bromide, or nickelocene can be directly or ultimately used to form anti-10 knock compounds such as those described in U.S. Pat. Nos. 3,086,035, 3,086,036, 3,086,037, 3,086,034, 3,086,984, 3,088,962, 3,088,963, 3,097,224, 3,097,225, etc.

The process of Example 2 can be used to treat solutions having in grams per liter:

nickel — 40 — 50  
cobalt — 0.7 — 1  
copper — 5 — 10  
ammonium sulfate — 120 — 180  
free ammonia — 85 — 100

Likewise, solutions having greater or lesser quantities of these substituents can be so treated.

Likewise, the process of the preceding example can be used to treat concentrates having nickel 10 percent, cobalt 0.5 percent, copper 2 percent, iron 38 percent, sulfur 31 percent and rock 14 percent by leaching such a solid pentlandite flotation concentrate with aerated ammonia and then treating the concentrate with synthesis gas under conditions as set forth in the preceding example.

Similarly, the procedure of the above example can be employed using a temperature of from 100° to 250°C., a H<sub>2</sub> pressure of from zero to 1,200 psig., a carbon monoxide pressure of from 200 to 1,200 psig., a time of from 1 to 4 hours, an amount of organic solvent (per unit volume of aqueous solution) of from 0.1 to 2.0, said solvent being selected from ligroin, n-octane, kerosene, n-nonane, and cyclohexane.

The procedure of the above examples can be extended to recovery of Ni, Cu, Co, Fe and precious metals. Thus, a sulfide concentrate containing these metals is smelted in air in a smelting furnace. Iron values can be recovered as known in the art and separated from a matte containing (some iron), nickel, copper, cobalt, and precious metals.

The matte is subjected to a pressure oxidation to yield soluble ammine sulfates of nickel, cobalt, and copper.

Iron values and precious metals are in the residue. 50 The precious metals are recovered as known in the art. The ammine sulfates are treated as in the previous examples to recover and separate copper, nickel, and cobalt.

55 The use of a catalyst for the formation of nickel carbonyl is a preferred embodiment of the invention and is illustrated by the following examples.

#### EXAMPLE 3

60 To a reaction vessel equipped with a stirrer was added 327 millimoles ammonium hydroxide (13.6 molar solution), 54.5 millimoles NiSO<sub>4</sub>, enough water to make a total volume of 100 ml. and then 10 ml. of heptane. The reaction vessel was closed and sealed, pressure lines were connected and the vessel flushed with nitrogen. After pressuring with nitrogen to 60 psig., the autoclave was heated to 150°C. On reaching temperature equilibrium, the reaction vessel was pres-

sured further to about 600 psig. with carbon monoxide. The reaction was continued for 3 hours. The total pressure drop in the reaction was 235 psi. After rapid cooling, the autoclave was vented.

The organic layer was separated. The amount of nickel carbonyl was determined by decomposition with bromine. The yield of nickel carbonyl was 30 percent. The aqueous phase contained unreacted nickel sulfate corresponding to 51 percent of the amount charged.

The following table shows effect of the addition of cyanide ion in the form of potassium cyanide, KCN. The reaction procedure is substantially the same as in Example 3 above. The various Examples 4-9 illustrate the effectiveness of the addition of a small amount of cyanide ion to the reaction mixture. Further, the catalysis by cyanide ion is not affected to any substantial extent by the presence of other metal ions.

TABLE I

[Cyanide-Catalyzed Reduction of Nickel, Cobalt, and Copper Sulfates]

|                                                | Example No. |     |     |      |     |      |
|------------------------------------------------|-------------|-----|-----|------|-----|------|
|                                                | 4           | 5   | 6   | 7    | 8   | 9    |
| <b>Reaction variables:</b>                     |             |     |     |      |     |      |
| Initial molar ratios:                          |             |     |     |      |     |      |
| NiSO <sub>4</sub> <sup>1</sup>                 | 9           | 110 | 110 | 110  | 101 | 110  |
| CoSO <sub>4</sub>                              |             |     |     |      | 12  | 12   |
| CuSO <sub>4</sub>                              |             |     |     |      | 27  | 27   |
| KCN                                            | 1           | 1   | 1   | 1    | 1   | 1    |
| Total pressure drop, p.s.i.                    | 395         | 410 | 410 | 425  | 400 | 315  |
| Reaction time, hrs.                            | 1.5         | 2.2 | 2.2 | 2.5  | 3.0 | 3.0  |
| Duration of gas uptake, hrs.                   | 0.75        | 1.8 | 1.8 | 2.5  | 3.0 | 3.0  |
| Results percent:                               |             |     |     |      |     |      |
| Recovered:                                     |             |     |     |      |     |      |
| NiSO <sub>4</sub> <sup>1</sup>                 | 4.8         | 1.9 | 1.9 | 2.4  | 8.8 | 30.8 |
| CoSO <sub>4</sub> <sup>2</sup>                 |             |     |     | 68.3 |     | 74.7 |
| CuSO <sub>4</sub>                              |             |     |     | 37.6 |     | 47.2 |
| Conversion <sup>4</sup> to Ni(CO) <sub>4</sub> | 90          | 98  | 98  | 94   | 92  | 72   |
| Conversion <sup>4</sup> to Cu metal            |             |     |     | 63   |     | 53   |

<sup>1</sup> 54.5 mmoles of NiSO<sub>4</sub> used in each run. The metal sulfate-ammonia ratio was 1:6 in each run. Total volume of each run was 100 ml. of aqueous phase and 10 ml. of heptane. All runs were carried out at 150°C. and 600 p.s.i. initial carbon monoxide pressure. Examples 4-9 were repressed three times back to 600 p.s.i.

<sup>2</sup> Gas was still being taken up very slowly when reaction was stopped.

<sup>3</sup> The amount of cobalt found in aqueous solution.

<sup>4</sup> Mmoles product found over mmoles of starting metal sulfate.

## EXAMPLE 10

The procedure of Example 9 is repeated except that the molar ratio of cyanide ion to metal is 1:1. The results obtained from such a reaction are similar to those of Example 9.

Similar results are obtained when the reaction is run under a carbon monoxide pressure of 400 psi. The reaction vessel may be repressed at regular intervals to maintain the carbon monoxide at about this level. Also, petroleum ether can be used for the solvent to extract the nickel carbonyl.

## EXAMPLE 11

The reaction vessel of Example 3 is filled according to the procedure of Example 1 with 327 mmoles of ammonium hydroxide, 54.5 mmoles of nickel sulfate, 13.6 mmoles of copper sulfate, enough water to make 100 ml. total volume, and then 10 ml. of heptane. Cyanide ion in the form of HCN gas is added to the reaction mixture in an amount sufficient to make the molar ratio of cyanide ion to metal of 1:6. The reaction vessel is pressured to 2,500 psig. with synthesis gas and heated to 150°C. The reaction is stopped after three hours and the products analyzed. The yield of neckel carbonyl is about 75 percent and about a 50 percent yield of copper metal is obtained.

Similar results are also obtained when the catalyst concentration of cyanide ion is about 0.1 mole percent based on the amount of nickel present.

## EXAMPLE 12

The process of Example 3 is repeated except that cyanide ion catalyst at a concentration of about 10 mole percent based on nickel is added. The rate of nickel carbonyl formation is increased by a factor of 10, and high yield of nickel carbonyl is obtained.

Similar results are obtained in this process using nonane as the hydrocarbon solvent. Also, the addition of cyanide ion in the form of NaCN brings similar results.

Similar results to those above are obtained when a nickel sulfide-containing ore concentrate is mixed with aqueous ammonia, aerated, and then contacted with carbon monoxide at a pressure of 600 psig. and a temperature of 100°C. in the presence of cyanide ion catalyst.

## EXAMPLE 13

Using the procedure of Example 3, a typical sulfide ore from Maine is concentrated by known methods to give a nickel-containing sulfide ore concentrate having the following analysis: Ni — 8.75%, Fe — 44.15%, Co — 0.85%, Cu — 0.73%, S — 34.24%, insol. — 5.64%, trace metal — 3.36%.

This concentrate is mixed with aqueous ammonia, NH<sub>4</sub>OH, and aerated according to known procedures. The aeration of the ammoniacal solution precipitates out iron as hydrated ferric oxide. Many other trace metal values are insoluble in NH<sub>4</sub>OH and, after these are removed, the Ni, Co, and Cu values are left in the ammonia leach solution as the ammonium sulfate complexes. The ammonium concentration in this solution is adjusted to give a NH<sub>4</sub>OH to nickel ratio of about 4:1 or 6:1 as desired.

To the solution is now added KCN in molar ratio of 110:1 NiSO<sub>4</sub>:KCN, heptane to form an organic layer on top. The vessel is sealed and pressured with carbon monoxide to 1,600 psig. and the temperature is maintained at 150°C. for three hours. When the vessel is vented, the organic layer is drawn off and the ammoniacal solution is removed. Metallic copper left in the bottom of the reaction vessel is removed from the reaction vessel.

Recovery of metal values is as follows: Cu — 53%; Ni — 72%, (as Ni(CO)<sub>4</sub>), Co — 74.7% (as CoSO<sub>4</sub>).

Another embodiment of this invention comprises the discovery that nickel carbonyl catalyzes the formation of copper from ammoniacal solutions of copper ammines. Thus, when treated with carbon monoxide, ammoniacal solutions of copper salts will give copper metal. When the same reaction conditions are employed — together with nickel carbonyl present in the system — the yield of copper metal is increased. This is demonstrated by the following example.

## EXAMPLE 14

A glass liner of a rocking autoclave was charged with 9.99 g. of CuSO<sub>4</sub>·5H<sub>2</sub>O, 16 ml. of concentrated ammonium hydroxide, and 35 ml. of water. The autoclave was pressured with 600 psig. of carbon monoxide and 600 psig. of hydrogen. The resultant mixture was heated for 2 hours at 150°C.

The resultant reaction mixture consisted of a colorless aqueous phase (which turned deep blue on exposure to air) and copper metal. The metal was filtered off, washed with aqueous ammonia, water and methanol. After drying in vacuo, the product copper weighed 0.56 g. (a 22 percent yield).

In another run, the glass liner was charged with 5.0 g. (20 mmoles) of  $\text{CuSO}_4 \cdot 5\text{H}_2\text{O}$ , 5.25 g. (20 mmoles)  $\text{NiSO}_4 \cdot 6\text{H}_2\text{O}$ , 16 ml. of concentrated ammonium hydroxide, 35 ml. of water and 10 ml. of heptane. The autoclave was pressured with 600 psig. each of hydrogen and carbon monoxide and heated 2.5 hours at 150°C. The resultant reaction mixture consisted of an aqueous layer, copper metal, and a colorless organic layer.

The copper metal was removed by filtration, washed and dried in vacuo. The amount of copper was 0.74 10 grams, a 58 percent yield.

The nickel yield — determined by treatment of the heptane layer with bromine in  $\text{CCl}_4$  was 52 percent. Similar results are obtained when the heptane is omitted.

A copper sample obtained by the procedure above wherein nickel was present in the reaction mixture contained 0.01 to 0.1 percent nickel.

#### EXAMPLE 15

A glass liner was charged with 5.0 g., 20.0 mmoles  $\text{CuSO}_4 \cdot 5\text{H}_2\text{O}$ , 5.25 g., 20.0 mmoles  $\text{NiSO}_4 \cdot 6\text{H}_2\text{O}$ , 21 ml. 320 mmoles concentrated  $\text{NH}_4\text{OH}$ , 25 ml. water, and 10 ml. heptane. The autoclave was pressured with 640 psi. hydrogen and 1,200 psi. carbon monoxide, then heated 2.0 hours at 150°C. The reaction mixture consisted of a colorless upper phase, metallic copper, and a light blue aqueous solution. The heptane phase was siphoned off and combined with subsequent heptane extracts of the aqueous phase. The organic solution was treated with excess bromine in carbon tetrachloride. The resulting mixture was filtered, washed with carbon tetrachloride, and dried. This gave 2.55 g. of light yellow-brown powder, identified as nickel bromide. The amount isolated corresponded to 11.7 mmoles  $\text{Ni}(\text{CO})_4$ , 58 percent yield based on starting  $\text{NiSO}_4$ .

Copper metal was isolated as above. The yield was 0.90 g. 14.2 mmoles (71 percent based on starting  $\text{CuSO}_4$ ). The above example can be repeated by using: 40 copper concentrations of from 0.001 grams per liter to saturated solution, nickel concentrations of from 0.001 grams per liter to saturated solution, ammonia concentrations of from 1 to 10 moles per 45 mole of metal, hydrogen pressures of from zero to 1,200 psig., temperatures of from 100° to 250°C.

However, it should be pointed out that the copper concentration is not critical. In addition, preferred copper concentrations are from 1 to 100 grams per liter. Preferred nickel concentrations are from 1 to 150 grams per liter. Preferred ammonia concentrations are within the range of from 1 to 10 moles per mole of metal. Preferred carbon monoxide pressures are from 200 to 400 55 psig. A preferred temperature range is from 100° to 200°C. Reaction times are not critical, times of 1 to 4 hours are usually sufficient. The presence of an immiscible organic solvent is not essential. However, because this embodiment lends itself to be an integral feature of a method for separation of copper metal from nickel carbonyl, it is usually preferred to carry out this embodiment in the presence of a solvent for nickel carbonyl. Solvents for this purpose and amounts thereof have been set forth above.

The nickel carbonyl need not be formed in situ. Rather, preformed nickel carbonyl can be added to the reaction mixture.

Another embodiment of this invention is the catalytic

5

effect of manganese carbonyl in the production of copper metal from carbon monoxide reduction of ammoniacal copper ammine solutions.

This is illustrated by the following example.

#### EXAMPLE 16

A glass liner of a rocking autoclave of roughly 300 ml. capacity was charged with

$\text{CuSO}_4 \cdot 5\text{H}_2\text{O}$  — 9.9 g.

$\text{Mn}_2(\text{CO})_{10}$  — 0.80 g.

Conc.  $\text{NH}_4\text{OH}$  — 16 ml.

Water — 35 ml.

n-Heptane — 10 ml.

The autoclave was pressured with 600 psi of hydrogen

15 and 600 psi of carbon monoxide, then heated 2.5 hours at 150°. The reaction mixture consisted of a colorless aqueous phase, metallic copper, solid  $\text{Mn}_2(\text{CO})_{10}$ , and a yellow organic phase. The heptane layer was siphoned off, and the remaining catalyst was extracted 20 with heptane and ether. Work up of the organic extracts gave 0.59 g.  $\text{Mn}_2(\text{CO})_{10}$  (74 percent recovery). Metallic copper was filtered off, washed with aqueous ammonia, water, and methanol. After drying in vacuo, 1.03 g. of copper (16.2 mmoles, 40.5 percent yield) 25 was obtained.

The preceding experiment was repeated using the same reaction conditions and the same quantity of reagents, but leaving out  $\text{Mn}_2(\text{CO})_{10}$  and heptane. There was obtained 0.56 g. 8.9 mmoles of copper metal, representing 22 percent yield. The aqueous phase of the reaction was colorless, but turned to deep blue color when exposed to air.

Because  $\text{Mn}_2(\text{CO})_{10}$  is a solid, it is preferred that the process be conducted in the presence of an organic solvent. In contrast,  $\text{Ni}(\text{CO})_4$  is a liquid and no solvent is required for it to render catalysis of copper metal preparation.

The above example can be repeated — and increased yields of copper obtained — by using:

40 copper concentrations of from 0.001 grams per liter to saturated solution,

manganese carbonyl copper ratios of from 0.001 to 0.5,

ammonia concentrations of from 1 to 10 moles per mole of metal,

hydrogen pressures of from 100 to 1,200 psig., carbon monoxide pressures of from 200 to 1,200 psig.,

temperatures of from 100° to 250°C.

50 However, it should be pointed out that the copper concentration is not critical. In addition, preferred copper concentrations are from 1 to 30 grams per liter. Preferred manganese carbonyl to copper ratio is from 0.01 to 0.4. Preferred ammonia concentrations are within the range of from 2 to 4. Preferred carbon monoxide pressures are from 200 to 400 psig. A preferred temperature range is from 150° to 200°C. Reaction times are not critical; times of 1 to 4 hours are usually sufficient.

60 Another embodiment is the catalytic effect of cobalt carbonyl in the production of copper metal from carbon monoxide reduction of ammoniacal copper ammine solutions. For example, similar results to those obtained by manganese carbonyl catalysis in Example 16 are obtained when cobalt carbonyl is substituted for the manganese carbonyl.

65 The following experiments are an indication that manganese carbonyl also catalyzes the formation of nickel carbonyl.

## EXAMPLE 17

The glass liner was charged with 10.5 g. 40 mmoles  $\text{NiSO}_4 \cdot 6\text{H}_2\text{O}$ , 0.80 g., 2.05 mmoles  $\text{Mn}_2(\text{CO})_{10}$ , 21 ml. conc.  $\text{NH}_4\text{OH}$  (c.a. 320 mmoles), 25 ml. water, and 10 ml. heptane. The autoclave was pressured with 820 psi  $\text{H}_2$  and 1,300 psi  $\text{CO}$ , then heated 2.5 hours at 150°, cooled, and vented through a dry ice trap. The reaction mixture consisted of a blue aqueous phase and a yellow organic phase. The heptane layer was siphoned off and the aqueous phase was extracted with about 30 ml. of heptane-hexane solution. The combined organic solution was distilled in vacuo into a dry ice-cooled receiver. Work-up of the distillation residue gave 0.53 g., 1.36 mmmole  $\text{Mn}_2(\text{CO})_{10}$ , representing 67 percent recovery. The distillate, containing  $\text{Ni}(\text{CO})_4$ , was treated at -76°C. with bromine-carbon tetrachloride solution until no more gas was evolved and the mixture contained excess of bromine. The suspension was filtered and washed with carbon tetrachloride. After drying in vacuo, 5.93 g. of nickel dibromide was obtained. Thus, the yield of nickel carbonyl was 27.1 mmoles, or 68 percent.

The amounts of starting materials used were the same as in the preceding experiment, except that no  $\text{Mn}_2(\text{CO})_{10}$  was added in this case. The autoclave was pressured with 800 psi  $\text{H}_2$  and 1,200 psi  $\text{CO}$  and heated 2.5 hours at 150°C. Following the same work-up procedure, 4.86 g. of  $\text{NiBr}_2$  was obtained. This corresponded to 22.2 mmoles of  $\text{Ni}(\text{CO})_4$ , 56 percent yield.

As with all processes of this invention — described and illustrated by the above description and examples — the processes of the aforesaid examples are not critically dependent on use of n-heptane. When an essentially water-immiscible solvent is used, it may be any solvent for nickel carbonyl. For economic reasons, aliphatic hydrocarbon materials are preferred solvents. To facilitate  $\text{Ni}(\text{CO})_4$  stripping the solvent preferably has a boiling point of at least about 36°C. There is no critical upper limit in boiling point of solvent.

From the foregoing description, it can be readily seen that the process of this invention is highly flexible. Thus, any method for obtaining nickel and its associated metals in the desired form for carbonylation may be used. A feature of this invention is, therefore, the combination of various pyrometallurgical, hydrometallurgical, vapormetallurgical, and physical separation processes with carbonylation to obtain and separate nickel and its associated metals. Indeed, such combination results in improved processes for winning nickel by advantageously using proven "front-end" processes in handling various types of ores most economically, dissolving or partially dissolving the nickel values in an aqueous ammonium salt or ammonium hydroxide solution and contacting the solution with a carbon monoxide-containing gas under conditions whereby the nickel values are reduced to form nickel carbonyl, copper values are precipitated as metallic copper, and cobalt values remain in aqueous solution as a cobalt carbonyl anion from which it is readily recovered by oxidation to hydrated cobalt oxide. Thus, the overall process effects removal of nickel and those associated metals from the material provided by the front-end process.

The wide applicability of such improved processes is illustrated by combining the above-described reductive carbonylation process with a sulfide or oxide ore leaching process, a ferronickel process, a blast furnace or converter matte process using either sulfide or oxide

ores or even a scrap metal recovery process. As a result of such improved processes, substantial savings in operational steps, processing costs, and capital investment are realized.

- 5 One currently employed process as schematically diagrammed in FIG. 2A shows a process employing crushing and grinding, drying the ore to prepare a material of suitable size, partially reducing the ore to the metals, cooling the reduced ore under non-oxidizing 10 conditions, oxidatively leaching the reduced ore with aqueous ammonia and carbon dioxide to dissolve nickel and cobalt as their carbonates. The leach solution is then boiled to concentrate the solution, recover ammonia values, and precipitate basic nickel carbonate. 15 The basic nickel carbonate is then sintered to produce a nickel oxide product.

FIG. 2B shows the improved process combining carbonylation after the oxidative leach. Such an improved process allows recovery of nickel metal and, in addition, cobalt by a simpler process requiring fewer operations and less processing equipment. According to FIG. 2B, the steps of ore preparation (which include crushing, grinding and drying), reducing and cooling under non-oxidizing conditions are the same as the process of

- 25 FIG. 2A. However, the oxidative leach may be carried out under more strenuous conditions and significant amounts of cobalt, suppressed in the previous process, are now leached from the ore. The previous process having no easy method for separating cobalt finds 30 leaching of the cobalt a liability to the process. However, the process of this invention easily separates cobalt and, thus, it becomes an asset to the process. After leaching, the leach solution is subjected to carbonylation under conditions whereby nickel and cobalt tetracarbonyl compounds are produced. The nickel carbonyl is separated from the solution and the metal recovered from the carbonyl compounds. The cobalt is separated in a different manner. Thus, a preferred embodiment of this invention is a process for recovering 35 nickel values from lateritic nickel ores predominantly of the silicate type ore containing them, said process comprising:

- a. subjecting said ore to a reducing roast to convert 45 a substantial amount of said nickel to nickel metal;  
 b. cooling the reduced ore under non-oxidizing conditions;  
 c. oxidatively leaching said reduced ore with an aqueous ammoniacal ammonium carbonate solution by injecting an oxygen-containing gas into a slurry of 50 said reduced ore in said ammoniacal ammonium carbonate solution;  
 d. contacting the resultant leach solution containing nickel ammonium salt complexes with a carbon monoxide-containing gas under conditions whereby the nickel values are reduced to nickel carbonyl;  
 e. separating said nickel carbonyl from said leach solution; and  
 55 f. decomposing said nickel carbonyl to metallic nickel.

The lateritic nickel ore is prepared for reduction by crushing and drying. A first crushing, for example, in toothed roll crushers, breads up larger lumps of ore for 60 convenient drying in a concurrently oil-fired rotary drying kiln. Temperatures in the kiln range from about 1,900°F. at the entrance to about 250°F. at the exit. The dry ore averages about 1.4 wt.% nickel and 0.1

wt.% cobalt. The dried ore is then finely ground in hammer and ball mills and charged to the reduction furnace.

Reduction is carried out in a multiple hearth furnace using a producer gas and additional heat from combustion of fuel oil. A sufficiently low heating rate permits substantially complete reduction of nickel oxide to metal at less than 1,400°F. Reduction is carried out at this temperature to obtain the maximum amount of nickel as the metal and yet limit the amount of iron and other impurities such as magnesia in the product. The reduced ore is cooled under non-oxidizing conditions by discharging the furnace into cooling tubes rotating in a water bath. The temperature of the ore on exiting from the coolers is about 300°F. The ore is then placed in quench tanks containing an ammoniacal ammonium carbonate leach solution. The leach solution is made by injecting ammonia and carbon dioxide into water. High temperatures in the quench tank are prevented by pre-cooling the ammoniacal leach liquor in water-cooled heat exchangers. Such low temperatures minimize ammonia vaporization and deposition of scale.

From the quench tank, the ore is leached in aerating tanks by injecting an oxygen-containing gas, for example air, into the solution. The oxidation of nickel dissolves the nickel into the ammonia ammonium carbonate solution as a stable hexammine nickel carbonate complex. Also, the recovery process of this invention permits a deep leach which also dissolves the cobalt values in the ore. Iron deposits out as hydrated ferric oxide and can be removed as such from the leach tank.

The dilute leach solution discharges into a series of thickeners which serve to settle and remove the gangue. The supernatant washed leach liquor can then be passed into an autoclave for carbonylation. The essentially iron-free solution containing nickel and cobalt values is contacted with a carbon monoxide-containing gas. This operation is carried out as described above to produce nickel carbonyl and cobalt tetracarbonyl anion. Separating of nickel carbonyl from the leach solution can be carried out by extracting the nickel carbonyl into an essentially water-immiscible, substantially inert solvent for nickel carbonyl, thus concentrating the nickel carbonyl produced in the solvent, or when the reaction is essentially complete, additional amounts of carbon monoxide-containing gas may be passed through the carbonylated leach solution to vaporize the nickel carbonyl. The nickel carbonyl is then passed into a decomposition zone to obtain metallic nickel. Decomposition is readily accomplished thermally by known methods.

This embodiment of the invention can be illustrated in the following examples. Unless otherwise stated, all parts are by weight.

#### EXAMPLE 18

A solution of basic nickel and cobalt carbonates such as result from the oxidative leach step of the above process, was prepared by dissolving 51 parts of  $\text{NiCl}_2 \cdot 6\text{H}_2\text{O}$  and 10 parts of  $\text{CoCl}_2 \cdot 6\text{H}_2\text{O}$  in 100 parts of water. To this solution was added sufficient aqueous sodium hydroxide to precipitate the metals as  $\text{Ni(OH)}_2$  and  $\text{Co(OH)}_2$ . After filtration, washing, and resuspension in water, 90-100 parts of ammonium carbonate and 27 parts of concentrated ammonium hydroxide were added. The solution was stirred and warmed slightly to yield a blue solution of nickel and cobalt salts.

The blue solution was then vaporized under vacuum

at 35°-40°C. to decrease the volume of solution. Any precipitated solids were re-dissolved using enough aqueous ammonia so that the final solution analyzed as follows:

- 5      2 parts  $\text{Ni}^{++}$   
       0.2 parts  $\text{Co}^{++}$   
       100 parts  $\text{H}_2\text{O}$   
       2 parts  $\text{NH}_3$  (as concentrated ammonium hydroxide)  
 10     This solution, corresponding to an oxidative leach solution according to the above process, was placed in a reaction vessel equipped with a stirrer, a thermocouple, a pressure gauge, a gas inlet tube, and a vent gas discharge tube. To the solution was added 7 parts of heptane. The autoclave was sealed and pressured to 300 psi. with carbon monoxide. The stirrer was started and the temperature in the reaction vessel brought up to 125°C. The reaction was continued for 40 minutes with carbon monoxide pressure decreasing to 220 psi. indicating the carbon monoxide was absorbed in the reaction vessel contents. The stirrer was stopped and the reaction vessel cooled. The remaining carbon monoxide was vented and the reaction vessel was opened.

15     The contents of the reaction vessel has separated into two layers. The heptane layer was drawn off and the remaining aqueous layer was observed to have the blue color characteristic of nickel and cobalt salt solutions. Therefore, the reaction, was of low yield. The organic layer was, therefore, not analyzed for nickel carbonyl.

20     Several runs were carried out using the procedure of Example 18 except for the addition of catalyst and the reaction time. The results are shown in Table II below.

TABLE II

| Example No. | Catalyst, 1 M KCN, ml. | Temp., °C. | CO press., p.s.i. | Time, hrs. | CO abs., p.s.i. | $\text{Ni}(\text{CO})_4$ , percent |
|-------------|------------------------|------------|-------------------|------------|-----------------|------------------------------------|
| 19 -----    | 0                      | 125        | 300               | 1.3        | 88              | 45                                 |
| 20 -----    | 5                      | 125        | 300               | 1.8        | 285             | 97                                 |
| 21 -----    | 5                      | 125        | 300               | 0.3        | 215             | 97                                 |

35     It will be appreciated by skilled practitioners that the invention does not require a solvent for separation of nickel carbonyl. However, it is a preferred embodiment 45 of the invention that the contacting with the carbon monoxide-containing gas is carried out in the presence of an essentially water-immiscible, substantially inert solvent for nickel carbonyl whereby said nickel carbonyl formed is concentrated in said solvent. As stated 50 previously, the solvent can be any solvent meeting the above criteria. A preferred solvent is an aliphatic hydrocarbon.

55     Example 19 in Table II above shows that a catalyst is not necessary for converting nickel to nickel carbonyl with carbon monoxide. However, it is clear from Examples 20 and 21 that the presence of a catalyst is extremely beneficial. Therefore, it is a preferred embodiment of the invention that the contacting with the carbon monoxide-containing gas is carried out in the presence of a catalyst for the formation of nickel carbonyl. A preferred catalyst is cyanide ion. A most preferred catalyst concentration is from about 0.01 to about 1 mole of cyanide ion per mole of nickel present.

60     While the nickel carbonyl may be separated from the aqueous reaction phase, by carrying out the reaction in the presence of a solvent, the nickel carbonyl may also be separated from the leach solution by passing additional carbon monoxide-containing gas through the

leach solution, allowing the nickel carbonyl to vaporize into the carbon monoxide-containing gas and venting the carbon monoxide-containing gas into a decomposition zone wherein the nickel carbonyl is decomposed to metallic nickel.

The silicate-type lateritic nickel ores also contain recoverable amounts of cobalt. Therefore, it is a preferred embodiment of this invention to recover cobalt using the process of this invention. When the ore contains recoverable amounts of cobalt, the process comprises subjecting the ore to a reducing roast to convert a substantial amount of the nickel and cobalt to the metals. The reduced ore is then cooled under non-oxidizing conditions and oxidatively leached with an aqueous ammoniacal ammonium carbonate solution by injecting an oxygen-containing gas into a slurry of the reduced ore and then contacting the resultant leach solution containing nickel and cobalt ammine salt complexes with a carbon monoxide-containing gas under conditions whereby the nickel and cobalt values are reduced to nickel carbonyl and cobalt tetracarbonyl anion in the leach solution. Then, the nickel carbonyl is separated from the leach solution and decomposed to metallic nickel, as previously described. The cobalt tetracarbonyl anion in the leach solution is separated therefrom by injecting an oxygen-containing gas into the solution whereby cobalt is oxidized to hydrated cobalt oxide. The hydrated cobalt oxide precipitates and is filtered from the remaining leach solution. It is then heated at a temperature sufficient to drive off the waters of hydration to produce cobalt oxide. This can be sold as such or further processed by calcining in the presence of a reducing gas at a temperature sufficient to reduce cobalt oxide to metallic cobalt. By this process, substantially pure metallic cobalt containing very little nickel is produced.

In another preferred embodiment, the above process is further characterized by heating the leach solution formed in the oxidative leach step to drive off ammonia and  $\text{CO}_2$ , thus precipitating the nickel and cobalt values as basic nickel and cobalt carbonates. These are then mixed in aqueous ammoniacal ammonium carbonate, thereby forming a mixture in which the nickel values are more concentrated. This resulting concentrate is contacted with a carbon monoxide-containing gas to form nickel carbonyl and cobalt tetracarbonyl anion. Nickel and cobalt are then recovered as previously described. This process variation has the advantage of concentrating the metal values, recovering ammonia and  $\text{CO}_2$  values, and allowing close control of process variations at an intermediate point in the process. It also allows the ore beneficiation and leaching steps to be conducted at one location and the metal recovery process to be carried out at a remote location without having to ship large volumes of the pregnant leach solution.

#### EXAMPLE 22

A cut of a laterite ore body is mixed with similar cuts of the ore body by clamshell bucket cranes to prepare a feed of reasonably uniform composition. The mixed feed is size-reduced in toothed roll crushers to break up large lumps of ore and then dried in a concurrently oil-fired rotary drying kiln. The dried ore averages the following composition:

1.5% nickel  
0.1% cobalt  
38% iron  
8% magnesia

#### 14% silica

The dried ore is then finely ground in hammer and ball mills to about 90 percent 200-mesh before reduction. The ore is then reduced in a multiple hearth furnace with producer gas from anthracite coal. Additional heat from combustion of heavy fuel oil is added as required. A strong reducing atmosphere is maintained by burning the coal or fuel oil at 50 percent of the theoretical air requirements. The ore is fed into the top of the furnace and producer gas enters at the bottom. The reduction of nickel metal is completed before the temperature reaches 1,400°F. The residence time in the furnace is about 90 minutes and reduced nickel is discharged as an iron-nickel alloy into cooling tubes. The cooling tubes are maintained in a non-oxidizing atmosphere to prevent re-oxidation of nickel. The nickel-iron alloy and ore is discharged from the cooling tubes at 300°F. into quench tanks containing pre-cooled leach liquor. The quenched solution is 6.5%  $\text{NH}_3$ , 3.5%  $\text{CO}_2$ , and 1% Ni, and is adjusted to maintain a pulp density of about 20% solids. The slurry is passed into aerating tanks and oxygenated by air. Nickel is dissolved into the solution and iron converts to hydrated ferric oxide. The nickel is combined with ammonia in the ammonia-ammonium carbonate leach liquor forming the stable hexammine complex  $\text{Ni}(\text{NH}_3)_6^{++}$ . The aeration tank discharge is thickened and product liquor containing the dissolved nickel is sent to steam stripping. The residue is washed by counter-current decantation in a 14%  $\text{NH}_3$ , 8.5%  $\text{CO}_2$  solution to recover any nickel values. The residual slurry is steam stripped to recover ammonia and carbon dioxide values. The product liquor from the thickener is a nickel-enriched ammoniacal ammonium carbonate solution. Traces of iron and ore fines are removed by agitation with air in an aerating unit. A filter aid such as diatomaceous earth is added and the solution is filtered.

The clarified product liquor is charged to a pressure reaction vessel and potassium cyanide catalyst is added. The reactor is pressurized with carbon monoxide and heated to 125°C. producing  $\text{Ni}(\text{CO})_4$ . The vapors are vented to a thermal decomposition zone and the nickel carbonyl is decomposed to produce carbon monoxide and metallic nickel powder. Additional carbon monoxide is passed through the reactor to sweep out any remaining nickel carbonyl product. This is also decomposed to produce additional nickel. Care should be taken to avoid exposure to nickel carbonyl which is very toxic.

One skilled in the art will appreciate that the above process may be varied greatly and still accomplish the same result. For example, instead of leaching with ammoniacal ammonium carbonate, a solution of ammoniacal ammonium sulfate or chloride may be used. Further, after removing the iron, the pregnant leach solution may be steam-stripped to remove  $\text{NH}_3$  and  $\text{CO}_2$  and precipitate nickel and cobalt as their basic carbonates; i.e.,  $\text{Ni}(\text{OH})_2 \cdot \text{NiCO}_3$  and  $\text{Co}(\text{OH})_2 \cdot \text{CoCO}_3$ . These are then redissolved or slurried in aqueous ammoniacal ammonium carbonate and treated with carbon monoxide in the presence of catalyst to produce nickel carbonyl and cobalt tetracarbonyl anion. The advantage of this procedure is its ability to decrease the volume of the carbonylation charge, reduce the size of reaction equipment required, and allow any necessary adjustments to be made in the system.

The cobalt is recovered from the solution by injecting an oxygen-containing gas, preferably oxygen or oxy-

gen-enriched air, into the solution to oxidize the cobalt to hydrated cobalt oxide. After filtering, the solid hydrated cobalt oxide is heated to produce marketable cobalt oxide free of water of hydration. Metallic cobalt may be prepared by calcining the cobalt oxide in the presence of a reducing gas, preferably synthesis gas or hydrogen, to reduce cobalt oxide to metallic cobalt.

In another preferred embodiment, nickel and cobalt may be recovered by using the above processes.

Another preferred embodiment is the process combining a pressure acid leaching process with reductive carbonylation. One ore body especially suited for the acid leaching is found near Moa Bay in Cuba. The ore contains a high valence ratio of nickeliferous iron ore to serpentine ore, about 10 to 1. Hence, the amount of acid soluble magnesia is considerably lower than with the Nicaro ores. The absence of large amounts of magnesia makes the Moa Bay ore amenable to acid leaching.

A useful process for recovering nickel from the Moa Bay ore includes selective mining of the limonitic-type deposits, ore preparation, leaching, and nickel-cobalt sulfides recovery, and refining to pure nickel and pure cobalt. The ore is size-reduced in a screening and slurring plant using grizzlies to reduce the size of the ore to about 5-inch pieces, adding water to make a thin slurry and passing the ore through counter-rotating paddle mixers to break up agglomerated lumps of fine ore material. The slurry is further screened to remove material coarser than 20-mesh and the resultant slurry containing 30 percent solids is thickened in preparation for leaching.

The sulfuric acid leach is selective to nickel and cobalt because these metals are more soluble than iron at the elevated temperature and pressure at which the process is carried out. A 45 percent solids solution from the thickener is pumped into mechanically agitated preheater tanks which brings the temperature to 170°F. by direct steam absorption. The slurry is then fed by high pressure pumps to heaters where direct steam injection at 610 psig. heats the slurry to reaction temperature of 450°-500°F. The slurry then flows into four autoclaves in series where it is contacted with concentrated (98 percent) sulfuric acid. Agitation of the slurry is maintained by steam injection. Nickel ions form, consuming about one-third of the sulfuric acid. The remainder goes to free acid and tailings. Leaching time is about 1 to 2 hours, depending on temperature, acid concentration, and ore composition. The leach slurry is cooled to below 275°F. by heat exchange and flows into a flash tank where atmospheric steam is produced and then separated from the slurry. The leached slurry is washed and separated from the residual solids in standard thickeners using continuous countercurrent washing with a pregnant solution being de-

canted from the first thickener.

The pregnant solution is neutralized using calcium carbonate from the coral mud dredged out of Moa Bay and suitably prepared for such use by screening and washing. The processed coral mud analyzes better than 90 percent calcium carbonate and completely reacts with the free acid in the pregnant solution to precipitate gypsum.

Prior to the present invention it was then necessary to preheat the neutralized solution to about 170°F. by steam and then pump it to the precipitation unit. Under 150 psig. and 245°F. the neutralized solution was contacted with gaseous high purity hydrogen sulfide. The

nickel and cobalt, as well as other metal impurities, were reacted to metal sulfides, which were precipitated from solution and sulfuric acid was produced.

The slurry resulting from H<sub>2</sub>S reaction was flashed to remove excess H<sub>2</sub>S and the sulfide slurry thickened and washed, forming a solid concentrate containing 99 percent of the nickel in the original leach solution.

The concentrate was treated by a refining process involving dissolution of the concentrate, precipitating the impurities, and extracting the pure metals. The concentrate was dissolved in sulfuric acid to form water-soluble sulfates by reacting with atmospheric oxygen under high pressure. The reaction is exothermic and produces sufficient heat to maintain the system at 350°F. and an operating pressure of 700 psig. The slurry discharged to a flash tank which in turn overflowed to a thickener where excess metal sulfides were collected and returned to the feed. The leach liquor was then pumped to a precipitation tank where ammonia was added with aeration to precipitate iron, chromium and aluminum as their hydroxides at atmospheric pressure and 180°F. The precipitate was filtered and redissolved to recover nickel values. The clarified solution from the precipitation reactor was reneutralized with ammonia to bring the pH to 5.0. The clarified product liquor was then treated with sulfuric acid and hydrogen sulfide to precipitate copper, lead and zinc as sulfides. On filtration, the filtrate containing nickel and cobalt sulfates was fed to the nickel recovery unit.

Nickel powder was obtained by reducing nickel sulfate with hydrogen at elevated temperature and pressure. Pure nickel was selectively precipitated so long as the ratio of nickel to cobalt remained high. The reduction step yields about 90 percent of the nickel values as nickel powder which contains about 0.1 percent cobalt. The powder was marketed as such or briquetted and sintered.

The many and complicated steps required by the process described above are greatly decreased when the front end of the process up through the dissolution of the nickel in the concentrated sulfuric acid is combined with reductive carbonylation metal recovery method. Consequently, a great saving in capital investment and processing cost is realized.

Therefore, a preferred embodiment of this invention is a process for recovery of nickel from laterite ores predominantly of the limonitic type, said process comprising:

- a. leaching said ore with sulfuric acid at elevated temperature and pressure;
- b. neutralizing the free acid in the resultant nickel-containing leach solution;
- c. adding ammonia to form a basic ammoniacal leach solution;
- d. contacting said basic leach solution with a carbon monoxide-containing gas under conditions whereby the nickel values are reduced to form nickel carbonyl;
- e. separating said nickel carbonyl from said basic leach solution; and
- f. decomposing said nickel carbonyl to metallic nickel.

One skilled in the art will appreciate a number of variations in the process which may effect a savings of raw materials and processing costs without departing from the above process to any great degree. As has been earlier described, the contacting with carbon monoxide may be carried out in the presence of an es-

sentially water-immiscible, substantially inert solvent for nickel carbonyl whereby the nickel carbonyl is concentrated in the solvent. Any of the solvents hereinabove described may be utilized, but a most preferred solvent is an aliphatic hydrocarbon such as hexane, heptane, octane, nonane, decane, and the like.

A further preferred embodiment of the above process is the use of a carbon monoxide-containing gas selected from the group consisting of synthesis gas and carbon monoxide.

A further preferred embodiment of the above process is characterized by carrying out the carbon monoxide-contacting of the above process in the presence of one of the previously described promoters; e.g., an amount of cyanide ion sufficient to catalyze the formation of nickel carbonyl. A most preferred amount of cyanide ion is present at a ratio of from 0.01 to 1 mole of cyanide ion per mole of nickel. The above catalyzed process may be carried out in the presence of a solvent as described above for separating the nickel carbonyl, or separation of nickel carbonyl may be effected by sweeping the reactor with a carbon monoxide-containing gas. Thus, a preferred embodiment of this invention is the separation of nickel carbonyl from the basic leach solution in step (e) above by passing a carbon monoxide-containing gas through the basic leach solution allowing nickel carbonyl to vaporize into the carbon monoxide-containing gas and subsequently passing the carbon monoxide-containing gas into a thermal decomposition zone wherein nickel carbonyl is decomposed to produce metallic nickel and carbon monoxide.

Cobalt metal values, found in conjunction with nickel may also be recovered by employing the above pressure leach with sulfuric acid according to the process of this invention. Therefore, a preferred embodiment of this invention is a process for recovery of nickel and cobalt from lateritic nickel ores predominantly of the limonitic type, wherein the ores contain recoverable amounts of cobalt, said process comprising:

- a. leaching said ore with sulfuric acid at elevated temperature and pressure;
- b. neutralizing the free acid in the resultant nickel and cobalt-containing leach solution;
- c. adding ammonia to form a basic ammoniacal leach solution;
- d. contacting said basic leach solution with a carbon monoxide-containing gas under conditions whereby the nickel and cobalt values are reduced to form nickel carbonyl and cobalt tetracarbonyl anion;
- e. separating said nickel carbonyl from said basic leach solution;
- f. decomposing said nickel carbonyl to metallic nickel;
- g. separating said cobalt from said basic leach solution by injecting an oxygen-containing gas into said solution whereby said cobalt tetracarbonyl anion is oxidized to hydrated cobalt oxide, and
- h. heating said hydrated cobalt oxide at a temperature sufficient to drive off the waters of hydration to produce cobalt oxide.

Although cobalt oxide is a marketable product, the metallic cobalt is a more valuable and salable product. This can be easily produced from cobalt oxide by calcining the cobalt oxide in the presence of a reducing gas; i.e., carbon monoxide or hydrogen, at a temperature sufficient to reduce the cobalt oxide to substan-

tially pure metallic cobalt and, therefore, such a step is a preferred embodiment of the invention.

The sulfuric acid pressure leaching process combined with reductive carbonylation is illustrated in the following example.

#### EXAMPLE 23

A nickel laterite ore of predominantly limonite is screened and ground to produce material less than 20-10 mesh and then water is added to make a slurry of 30 percent solids. The slurry is fed to a preheater and heated to 170°F. with steam and then by high pressure pumps is to heaters, where direct steam injection at 610 psig, heats the slurry to 500°F. The slurry flows by gravity into four leaching autoclaves in series where it is contacted with concentrated (98 percent) sulfuric acid for from 1 to 2 hours. Steam agitation is used to insure thorough contacting. The leached slurry is then cooled, steam is flashed off and the system is brought back to atmospheric pressure.

The resultant nickel-cobalt solution is separated from the residual solids in a series of six counter-current decantation operations in washing thickeners. The free acid remaining in the solution is then neutralized with calcium carbonate in the form of coral mud. The neutralization produces gypsum which is separated by counter-current decantation in another series of washing thickeners.

The neutralized leach liquor is then charged to an autoclave, KCN and kerosene are added and the reactor is pressurized to 300 psig. with carbon monoxide. The temperature is brought to 250°F. and the solution is mechanically agitated. After carbon monoxide pressure uptake ceases, the autoclave is cooled and vented to atmospheric pressure. The hydrocarbon layer is drawn off and distilled to separate nickel carbonyl and the kerosene solvent. The nickel carbonyl is obtained in good yield and can be converted to metallic nickel by thermally decomposing on pre-formed nickel nuclei.

The nickel carbonyl can also be recovered without the use of a solvent. In such a case, the reactor is swept with a carbon monoxide-containing gas and the nickel carbonyl vaporizes into the gas. The nickel carbonyl-containing gas is then passed into a thermal decomposition zone where it is decomposed to metallic nickel and carbon monoxide.

A major source of nickel prior to the discovery of the rich sulfide ore deposits in Canada was the laterite nickel ores of New Caledonia. These deposits continue to be mined, and although the richest of the ores has been taken, laterite nickel ores ranging from 1 to 5 percent nickel continue to yield high tonnages of nickel metal. Two processes were developed during the 19th century to recover nickel from these rich deposits — smelting to ferronickel and smelting to matte.

Blast furnaces were first used in smelting the ore to ferronickel. However, difficulties in refining the crude product to acceptably pure nickel metal caused producers to change to production of matte. Later, high demand for nickel alloy steels and improved impurity removal allowed a return to the simpler reduction of ores to ferronickel.

One process for smelting nickel laterite ores to ferronickel is illustrated in FIG. 3. FIG. 3 shows in Part A a schematic representation of ferronickel process. In general, the process includes the steps of ore preparation, drying, and preheating, smelting, desulfurizing,

blowing with oxygen, and casting into the refined ferronickel product.

The ore preparation consists of size reduction and classification and is usually accomplished by crushing and grinding or ball milling. The ore is screened to prepare a feed of uniform consistency. These operations are similar to those previously described and are well known in the art.

The uniform ore feed is then dried and dehydrated in concurrently fired rotary kilns which also serve the dual function of preheating the ore for smelting. The oil burners use 60 percent excess air to avoid clinker formation and assure adequate moisture removal by the gases. Drying removes the free moisture present in the ore feed at about 220°F. while dehydration removes the chemically combined moisture present as hydroxyl groups associated with the mineral lattice structure. On heating between 600° – 1,200°F. the hydroxyl groups decompose leaving some oxygen in the lattice structure while the rest of the hydrogen and oxygen combine, evolving as water vapor. About 20–30 percent of the original ore weight is lost as free moisture and about 12 percent is lost as combined moisture.

The kiln product is fed to the smelting furnace with coke and the crude ferronickel is taken from the furnace. Smelting may be carried out in blast furnaces, rotary kilns, or electric arc furnaces. Depending on the availability of cheap electric power, the electric arc furnace is preferred since it has the advantage of high, localized and controllable temperatures as well as being suited to treatment of oxide nickel ores.

Smelting causes the reduction of nickel and iron oxides by reaction with carbon to produce the metals and carbon monoxide. In addition, a number of side reactions occur. The major part of the reduction is coincident with melting of the ore. This is done in the presence of carbon, added as coke. Almost all of the nickel and cobalt are reduced to the metal, but iron reduction depends on the amount of carbon added. That portion of the iron which is not reduced to metal combines with the silica to form slag.

In electric arc furnace smelting, the furnace is usually operated on the "submerged arc" principle in which electrodes in contact with the slag form a circuit. Current passed through the circuit produces heat in the slag because of its resistance. The electrodes are typically carbon and the furnace is operated on three-phase power with six electrodes, a pair of which constitute one phase. The electrodes are consumed and are periodically replaced. A charge of kiln-dried calcine is fed into the top of the electric furnace and settles as an un-melted layer over the slag. Gradually the calcine settles into the slag as it melts and then separates into ferronickel matte and slag. The ferronickel being more dense settles to the bottom and both slag and ferronickel product are intermittently tapped. Since no fuel is combusted in the smelting operation, a smaller quantity of gases exit the electric furnace. Thus, dust and heat recovery problems are less complicated. While electric energy is usually more expensive than fossil fuel per unit of gross heating value, the high efficiency and excellent temperature control offer advantages which keep electric furnaces competitive.

The ferronickel can be refined by decreasing the sulfur content under reducing conditions and then removing other impurities under oxidizing conditions. The ferronickel is tapped from the electric furnace into a

ladle to which soda ash is added simultaneously. On entering the melt, soda ash (sodium carbonate) decomposes to sodium oxide and carbon dioxide. The sodium oxide reacts with sulfur and silicon in the melt forming a slag consisting of sodium sulfide and silicate. When the ladle fills, it is poured into a second ladle with the addition of more soda ash reducing the sulfur content of the ferronickel to about 0.02 percent. Temperature decline during desulfurization is prevented by blowing oxygen into the melt using an oxygen lance. The silicon oxidizes with generation of heat.

The desulfurized ferronickel is then converted by blowing air through the melt in two stages. Converting is an oxidation step used to reduce the impurities in molten metal melt. The ferronickel is added to a vertical side blown converter in which chromium and silicon are preferentially oxidized and form a slag which is skimmed. During the second stage, lime is added and unites with the phosphorus as calcium phosphate. A small amount of sand flux is added and the slag formed thereafter is skimmed off. The refined ferronickel is then cast into pigs and the slag is discarded. A typical analysis of the refined ferronickel is as follows:

29 percent nickel-cobalt

25 0.02 percent sulfur  
0.02 percent phosphorus  
0.02 percent carbon  
0.02 percent silicon  
balance — iron

30 The improved process of this invention is represented schematically by FIG. 3B. During the first portion of the process, it is similar to the above-described ferronickel process. Thus, the laterite ore is crushed and screened, kiln dried, preheated and smelted to produce 35 a crude ferro-nickel product. These operations are carried out as described above. When the crude ferronickel is tapped from the electric arc furnace, it is then granulated by passing the molten ferronickel into a water-quench forming granules of crude ferronickel 40 containing the impurities described above. This granulated material is then leached in an aqueous ammoniacal carbonate solution by injecting air or oxygen-enriched air into the leach solution. The nickel and cobalt values are selectively dissolved and iron is reacted 45 to hydrated ferric oxide and separated from the leach solution. The leach solution is then carried to a reductive carbonylation step such as previously described. In this step the leach solution is contacted with a carbon monoxide-containing gas, typically in the presence of 50 a catalyst for the formation of nickel carbonyl. The nickel carbonyl is separated from the leach solution and metallic nickel is recovered. Cobalt in the form of cobalt tetracarbonyl anion remains in the spent leach solution and can be separated and recovered therefrom.

55 Therefore, a preferred embodiment of this invention is a process for recovering nickel and cobalt from a ferronickel product, said process comprising oxidatively leaching said ferronickel product with an aqueous ammoniacal ammonium salt solution by injecting an oxygen-containing gas into a slurry of said ferronickel product in said aqueous ammoniacal ammonium salt solution. The resultant leach solution is contacted with a carbon monoxide-containing gas under conditions whereby the nickel and cobalt values are reduced to nickel carbonyl and cobalt tetracarbonyl anion. The nickel carbonyl is separated from the leach solution and decomposed to metallic nickel. The cobalt is sepa-

rated from the leach solution by injecting an oxygen-containing gas into the leach solution whereby the cobalt tetracarbonyl anion is oxidized to hydrated cobalt oxide and subsequently heated at a temperature sufficient to drive off the waters of hydration to produce cobalt oxide.

As described previously, the reductive carbonylation step can be carried out in the presence of a promoter such as cyanide ion in an amount sufficient to catalyze the formation of nickel carbonyl. A preferred concentration of cyanide ion is from 0.01 to about 10 moles of cyanide ion per mole of nickel present. Further, it is a preferred embodiment of this process to carry out the contacting with the carbon monoxide-containing gas in the presence of an essentially water-immiscible, substantially inert solvent for nickel carbonyl whereby the nickel carbonyl formed is concentrated in the solvent. Any solvent described previously may be used in this preferred embodiment. However, a most preferred solvent is a saturated aliphatic hydrocarbon. The aqueous ammoniacal ammonium salt solution in which the ferronickel is oxidatively leached is preferably an aqueous ammoniacal ammonium chloride, carbonate, sulfate or the like. A most preferred aqueous ammoniacal ammonium salt solution is aqueous ammoniacal ammonium carbonate. In lieu of forming nickel carbonyl in the presence of a solvent, the nickel can be separated from the leached solution by passing a carbon monoxide-containing gas through the leach solution allowing the nickel carbonyl to vaporize into the carbon monoxide-containing gas and subsequently passing the carbon monoxide-containing gas into a thermal decomposition zone wherein nickel carbonyl is thermally decomposed to metallic nickel.

The above process for producing nickel and cobalt from ferronickel can be illustrated by the following example.

#### EXAMPLE 24

A laterite ore from New Caledonia is screened to obtain material of the same size for further processing. Oversize pieces are crushed and returned to the screening unit. The screened ore is ball milled to prepare a fine charge for kiln drying. The finely ground ore is charged to a concurrently oil-fired rotary kiln to remove the free and combined moisture and preheat the charge for smelting. The highest kiln temperature is about 1,400°F. The kiln discharge, free of moisture, is fed through the top of an electric arc furnace with coke and the ore is melted and reduced to crude ferronickel and slag. The crude ferronickel is tapped into quench tanks containing an aqueous ammoniacal ammonium carbonate solution where it is granulated and the slurry is passed into an aerating unit where it is contacted with air. The nickel and cobalt values are extracted into the leach solution as the stable ammine complexes. Iron forms hydrated ferric hydroxide and is removed by a series of counter-current decantation washing thickeners. Other insoluble impurities such as chromium, silicon and phosphorous remain with the ferric hydroxide residue. Carbon is reacted to form carbon dioxide and dissolves or it falls out of the leach solution as insoluble clinkers and is removable with the residue.

The leach solution is fed into a pressure reactor with addition of cyanide ion catalyst and the reactor is pressurized with carbon monoxide to about 300 psig. On heating to about 250°F. with mechanical agitation, the

carbon monoxide is absorbed, forming nickel carbonyl and cobalt tetracarbonyl anion. Nickel carbonyl is vented to a thermal decomposition zone and decomposed to metallic nickel. A high yield of substantially pure metallic nickel is obtained.

The cobalt tetracarbonyl anion in the leach solution is oxidized to hydrated cobalt oxide and filtered from the spent leach solution. It is then heated to drive off the waters of hydration producing marketable cobalt oxide in good yield.

The above example may be carried out in the presence of a solvent for nickel carbonyl as described previously and separated therefrom to recover the nickel carbonyl. A preferred solvent is a saturated aliphatic hydrocarbon. Also, the cobalt oxide may be upgraded to metallic cobalt by calcining the cobalt oxide in the presence of a reducing gas. These and other process expedients may be employed without departing from the scope of this preferred embodiment.

The matte smelting process was derived from earlier experience in Europe when sulfide ores, the only known source of nickel, were obtained by smelting to matte. This technique of smelting in blast furnaces was applied to the oxide ores. The basic principle employs

the natural affinity of sulfur for metals as a means of separating the metals from the ore. Of course, the sulfide ores are themselves sulfur sources. However, the oxide ores require the addition of a sulfur source. Such a process is illustrated in FIG. 4A. The schematic diagram illustrates a process of crushing and screening a laterite ore, sintering with coke and smelting in a blast furnace with gypsum, the sulfur source, to produce an iron-nickel matte. The matte is then converted by air blowing to nickel sulfide matte which may either be cast into anodes for electro-winning of nickel or roasted in a two-stage process to a nickel oxide product. After briquetting and drying, the nickel oxide is reduced with charcoal to form nickel rondelles.

The crushing and screening of the oxide type ore is carried out as described previously using well-known techniques. Instead of kiln drying, however, this process removes free and bound moisture and agglomerates the ore fines by means of sintering on a travelling grate. In this respect, blast furnace smelting differs from practice using electric arc furnaces in that the fine ore particles must be agglomerated prior to charging to the blast furnace. Otherwise, they would be blown out of the vertical shaft of the blast furnace without reduction.

The crushing and screening of the oxide type ore is carried out as described previously using well-known techniques. Instead of kiln drying, however, this process removes free and bound moisture and agglomerates the ore fines by means of sintering on a travelling grate. In this respect, blast furnace smelting differs from practice using electric arc furnaces in that the fine ore particles must be agglomerated prior to charging to the blast furnace. Otherwise, they would be blown out of the vertical shaft of the blast furnace without reduction.

Sintering is typically used in conjunction with a pelletizer to agglomerate the fines. Ore material less than one-eighth inch in size is fed into a rotating drum or disc pelletizer and sprayed with a controlled amount of water. The rotation of the drum or disc causes tumbling ore particles to come into intimate contact, form seed particles, and then a "snowball" effect increases the size of the moist pellets. Pellets of 1½ inches in diameter are suitable for charging with the coarser ore to the sintering machine.

Sintering is effected on endless conveyors of linked grates sections or pallets into which the charge is fed. The pallets pass over a wind box and a downdraft of heated gases from a fuel burner is blown through the ore. In the sulfide ores, the sulfur is ignited and combustion is maintained by continuing to pass air through the ore. For the oxide ore, coke is added to the feed and its combustion continues the heating down the

length of the traveling conveyor. The roasting zone travels downward through the charge as the pallets move along the conveyor, bringing the charge to a temperature at which stickiness occurs because of incipient fusion. The fusion produces a strong, porous cake which is dumped at the end of the conveyor. Melting should be avoided because passage of air is impeded, interfering with sintering action.

The sintered ore is then charged to the blast furnace for reduction of the ore to matte and slag. The charge to the blast furnace is ore, coke, gypsum and limestone. As mentioned above, since oxide ores do not contain a source of sulfur to collect the metals, gypsum, hydrated calcium sulfate,  $\text{CaSO}_4 \cdot 2\text{H}_2\text{O}$ , is added to the charge. In addition to providing sulfur, the calcium oxide from reduction of  $\text{CaSO}_4$  with carbon monoxide serves as a flux material. Additional fluxing material in the form of limestone,  $\text{CaCO}_3$ , is used.

The charge is added at the top of the furnace and as it moves down the shaft, counter-current to hot reducing gas, it is heated, reduced, and melted to produce matte and slag. The major reactions are the reduction of iron and nickel oxides to the metals with either carbon monoxide or carbon. The calcium sulfate is reduced to the sulfide which in turn reacts with iron and nickel oxides to form iron and nickel sulfide, forming the molten matte. The slag is a calcium-iron magnesium-silicate. The composition of matte and slag is a balancing of the competing reactions determined by the amount of gypsum and coke used. With low gypsum and coke, a high nickel content matte is produced, but losses of nickel to the slag are also higher. With high gypsum and coke, the matte will have a greater iron and sulfur content with lower nickel losses, but a more costly converting operation to remove the iron.

The matte produced by blast furnace smelting is similar to that of the sulfide ores and is treated accordingly. The matte is charged to converters, usually the horizontal side-blown type, and blown with air to remove iron as slag. The converting procedure combines oxygen with the iron and sulfur to form iron oxides and sulfur dioxide. The sulfur dioxide passes off as a gas and the iron oxides react with added silica to form iron silicate slag. Thus, a nickel sulfide matte results which can be cast into anodes for electro-winning of nickel ore roasted with air to the nickel oxide and reduced to nickel.

The nickel matte from converters is granulated in water and contains about 78 percent nickel, 22 percent sulfur, and a small amount of impurities. The granulated matte is crushed and ground and then roasted in a two-stage process to remove the remaining sulfur. The two-stage roasting is carried out in a fluidized bed roaster and a rotary kiln. The nickel sulfide matte contains sufficient sulfur to support an exothermic reaction and, thus, the fluid bed roaster requiring no extraneous fuel source is used as the most efficient roasting method. When the sulfur has largely burned to  $\text{SO}_2$ , the roasted matte is fed to a countercurrently oil-fired rotary kiln to complete the roasting to nickel oxide. The nickel oxide is cooled and screened to make a uniform feed for briquetting prior to the final reduction to metallic nickel. The cooled nickel oxide is mixed with water and a binder material, such as starch and briquetted by reciprocating pistons into cylinders  $1\frac{1}{4}$  inches in diameter and  $\frac{3}{4}$  inch thick, called rondelles. The rondelles are dried and charged to a reducing re-

tort with charcoal. The rondelles descend from the top of the retort counter to a stream of producer gas and air which is introduced at several levels to regulate the temperature throughout the retort. The nickel oxide rondelles are reduced to nickel metal rondelles at  $2,400^\circ\text{F}$ . Magnetic separation removes the metal rondelles from excess charcoal from a gas-tight cooler at the bottom of the retort. The final product contains 99.5 percent nickel.

10 Using the above process as a preliminary treatment, a preferred process is illustrated in FIG. 4B. As in the above description of FIG. 4A, the ore is crushed, screened, sintered and smelted. The nickel-iron matte produced may then be further converted to a nickel sulfide matte or taken directly from the blast furnace and, after suitable crushing and grinding, is leached with an ammonium salt solution and carbonylated as described above. The nickel carbonyl is separated and nickel metal is recovered therefrom. Also, any cobalt 15 received may be reacted to form the metal or oxide from the tetracarbonyl anion produced. Thus, another preferred embodiment of the invention is the recovery of nickel from a nickeliferous laterite ore, said process comprising smelting the ore in a blast furnace with coke, gypsum and limestone to produce a matte containing nickel, iron, and sulfur, oxidatively leaching the matte with an aqueous ammoniacal ammonium salt solution by injecting an oxygen-containing gas into a slurry of said matte whereby the nickel values are selectively dissolved into the aqueous ammoniacal ammonium salt solution. The resultant leach solution is contacted with carbon monoxide-containing gas under conditions whereby the nickel values are reduced to form nickel carbonyl. The nickel carbonyl is separated 20 from the leach solution and decomposed to metallic nickel.

25 As previously described, the contacting of the leach solution with a carbon monoxide-containing gas is preferably carried out in the presence of an essentially water-immiscible, substantially inert solvent for nickel carbonyl whereby the nickel carbonyl formed is concentrated in the solvent. Any of the solvents previously described is suitable for use in this preferred embodiment. A most preferred solvent is a saturated aliphatic hydrocarbon. A preferred aqueous ammoniacal ammonium salt solution for the oxidative leach step is selected from the group consisting of aqueous ammoniacal ammonium chloride, carbonate, sulfate, or mixtures thereof. A most preferred aqueous ammoniacal ammonium salt solution is aqueous ammoniacal ammonium carbonate. Also, aqueous ammonium hydroxide may be employed as the leach solution. Another variation of this preferred embodiment is the precipitation of basic nickel carbonate from the leach solution and then mixing the precipitate with aqueous ammoniacal ammonium carbonate, thereby forming a mixture in which the nickel values are more concentrated. This procedure has the advantage of concentrating the nickel values. Thus, a preferred process of invention is further characterized by heating the oxidative leach solution to drive off ammonia and precipitate a substantial amount of the nickel values contained in the leach solution, separating the precipitated nickel values and then mixing them in an aqueous ammoniacal ammonium carbonate solution forming a mixture in which the nickel values are concentrated. The mixture is contacted with a carbon monoxide-containing gas to form nickel carbonyl and separating the nickel carbonyl from the mix-

ture. As previously described, this preferred embodiment may be further characterized by carrying out the contacting of the leach solution with a carbon monoxide-containing gas in the presence of one of the previously described promoters such as an amount of cyanide ion sufficient to catalyze the formation of nickel carbonyl. Another preferred process of this embodiment is characterized by carrying out the oxidative leach with an oxygen-containing gas selected from the group consisting of oxygen-enriched air and oxygen. A most preferred oxygen-containing gas is oxygen.

Instead of concentrating the nickel carbonyl formed in a solvent, the nickel carbonyl can be separated from the carbonylated reaction solution by passing a carbon monoxide-containing gas through said solution, allowing the nickel carbonyl to vaporize into the carbon monoxide-containing gas and subsequently passing the carbon monoxide-containing gas into a thermal decomposition zone wherein the nickel carbonyl is decomposed to metallic nickel.

Another preferred process of this embodiment is the recovery of cobalt in conjunction with the nickel metal. Thus, nickel and cobalt may be recovered from an oxide-type ore containing recoverable amounts of nickel and cobalt in a process comprising smelting the ore in a blast furnace with coke, gypsum, and limestone to produce a matte containing nickel, cobalt, iron, and sulfur; oxidatively leaching the matte with an aqueous ammoniacal ammonium salt solution by injecting an oxygen-containing gas into a slurry of the matte whereby the nickel and cobalt values are selectively dissolved in the aqueous ammoniacal ammonium salt solution. The resultant leach solution is contacted with a carbon monoxide-containing gas under reducing conditions to produce nickel carbonyl and cobalt tetracarbonyl anion. The nickel carbonyl is separated from the leach solution and decomposed to substantially pure metallic nickel. The cobalt is recovered from the leach solution by injecting an oxygen-containing gas into the solution whereby the cobalt tetracarbonyl anion is oxidized to hydrated cobalt oxide, and heating the hydrated cobalt oxide at a temperature sufficient to drive off the waters of hydration produces marketable cobalt oxide. Cobalt metal can be produced from the cobalt oxide by methods known in the art. Thus, a preferred process of this embodiment is characterized by calcining the cobalt oxide in the presence of a reducing gas at temperatures sufficient to reduce the cobalt oxide to substantially pure metallic cobalt.

One skilled in the art will appreciate that each of the preferred variations described above for the production of nickel metal by this embodiment can be applied to the preferred process for production of nickel and cobalt. Thus, the cyanide catalyst, the water-immiscible solvent, and the various aqueous ammoniacal ammonium salt solutions may be employed in the process for producing nickel and cobalt.

In addition to the preferred embodiment for producing nickel by smelting to nickel matte, it is a preferred process of this embodiment to convert the matte to a nickel sulfide matte by conventional converting procedures. Thus, after smelting, the nickel-iron matte may be converted by blowing with air or oxygen-enriched air in the presence of a siliceous flux at a temperature sufficient to at least maintain part of the matte in a molten state, thereby decreasing the iron and sulfur content of the matte. The nickel sulfide matte may then be

leached and carbonylated as described above. In this manner, recoverable amounts of cobalt may also be obtained. FIG. 4B schematically illustrates the variation in this preferred process by showing a broken line from the smelting step to the granulation step. Thus, the process of this embodiment employs an oxidative leach step and subsequent carbonylation after either the smelting or converting operation described above.

In the sulfide matte smelting process described in FIG. 4A, the matte was roasted and, thus, oxidized with air to produce nickel oxide which was subsequently briquetted and reduced with charcoal to nickel rondelles. Another preferred process of this embodiment is to employ a reductive carbonylation of the nickel oxide material produced from the two-stage roasting process described above. Thus, another preferred process of this invention is a process for smelting a nickeliferous laterite ore in a blast furnace with coke, gypsum, and limestone to produce a matte containing nickel, iron, and sulfur, converting the matte by blowing with air or oxygen-enriched air in the presence of a siliceous flux at a temperature sufficient to maintain at least part of the matte in a molten state, thereby reducing the iron and sulfur content of the matte. The converted matte is then contacted with an oxygen-containing gas under oxidative conditions at an elevated temperature sufficient to oxidize the matte substantially to nickel oxide. The nickel oxide is then dissolved or slurried in an aqueous ammoniacal ammonium salt solution. The resultant solution is contacted with a carbon monoxide-containing gas under conditions whereby the nickel values are reduced to form nickel carbonyl. The nickel carbonyl is then separated from the solution and decomposed to metallic nickel.

The preferred embodiments of utilizing a water-immiscible solvent, a cyanide catalyst, and an aqueous ammoniacal ammonium chloride, carbonate or sulfate leach solution may also be employed in this preferred process. Further, if the ore contains recoverable amounts of cobalt, it is a preferred process to recover the cobalt from the leach solution as cobalt oxide according to procedures described previously.

The blast furnace smelting of an oxide ore to a sulfide matte followed by reductive carbonylation is illustrated by the following example.

#### EXAMPLE 25

The process is carried out on a hydrated nickel-iron-magnesium silicate ore having a free moisture content of from 20 to 30 percent by weight and having an average analysis as follows:

2.8% nickel  
0.06% cobalt  
13% iron  
2% chromic oxide  
37% silica  
24% magnesia  
2% alumina  
12% loss on ignition

The ore is prepared for smelting by screening and crushing and then sintering on traveling grates. The sintered ore is charged with 500 pounds of coke, 175 pounds of gypsum, and 450 pounds of limestone per ton of dry ore to a blast furnace operating at about 2,500°F. and using preheated blast air at about 2 psig. and 1,600°F. The nickel recovery in the matte is about 90 percent of the nickel in the ore. Matte is tapped and

charged to a horizontal side-blown converter with silica in addition to recycled granulated slag. The converter is blown with air to oxidize iron selectively and slag it off as an iron silicate slag. As the blowing continues, the temperature decreases to about 1,950°F. and sodium sulfate is added to restore the pasty slag to more liquid form. The nickel sulfide matte containing about 0.1 percent iron is then granulated by pouring the converter matte into quench tanks. The granulated matte is then slurried in an aqueous ammoniacal ammonium carbonate solution. The resulting slurry is fed into aerating units and nickel and cobalt selectively dissolve into the solution while the iron remaining is reacted to hydrated ferric hydroxide. The leach solution containing dissolved nickel and cobalt values is separated in a series of counter-current decantation thickeners from the residue which is washed to recover any soluble nickel and cobalt values leaving with the residual slurry. The leach solution is then fed to a pressure reactor with the addition of potassium cyanide as a catalyst and the reactor is pressured with carbon monoxide at about 300 psig. The leach solution is heated to about 250°F. and agitated mechanically. After 2 hours, the reactor is cooled and vented to a thermal decomposition zone where the nickel carbonyl formed during the reaction is decomposed to metallic nickel. Additional carbon monoxide is passed through the reaction solution to sweep out all of the nickel carbonyl.

The cobalt tetracarbonyl anion in solution is charged to aerating units and air is injected into the solution to form hydrated cobalt oxide. The hydrated cobalt oxide is then heated in a rotary kiln to dry and dehydrate the cobalt oxide.

Both nickel metal and cobalt oxide are recovered in good yield from this process. Cobalt metal may be produced by further operations to reduce the cobalt oxide with hydrogen to metallic cobalt.

Similar results are obtained when the oxidative leach is carried out with aqueous ammoniacal chloride, sulfate or mixtures thereof. Further, aqueous ammonium hydroxide may also be employed in this process. Also, the carbon monoxide may be replaced with synthesis gas. Further, a precipitation step may be added after the oxidative leach to form insoluble basic nickel and cobalt carbonates. These are redissolved or slurried in ammoniacal ammonium salt solution and carbonylated as described above. This step has the advantage of adjusting the volume of the charge and concentrating the nickel and cobalt salts therein to utilize processing equipment of smaller throughput more efficiently. The catalyst may be added as HCN gas which is dissolved in the leach solution prior to carbonylation with similar results.

Another preferred embodiment of this process is illustrated in FIG. 5 which is a schematic representation of a hydrometallurgical process for winning nickel from a sulfide ore. FIG. 5A is a schematic diagram of a known process for obtaining nickel from a sulfide ore by crushing and grinding the ore to appropriate size, beneficiating the ore to produce a nickel concentrate containing about 10 percent nickel, performing an oxidative leach on the nickel concentrate by reacting with air and ammonia. Since the leach operation also carries over some copper, it is removed in a two-stage operation by first boiling the leach solution with steam and sulfuric acid and then adding H<sub>2</sub>S in a stripping step. The copper removed as copper sulfide is sent to a

smelter for recovery. The copper-free solution is then subjected to oxyhydrolysis which is a combination of air oxidation and hydrolysis of the nickel at 425°F. and 600 psig. The nickel is then reduced with hydrogen to the metal and obtained as a nickel powder slurry. It is usually washed, dried and briquetted and sold as such.

In contrast to the numerous processing steps and the resultant expense in capital investment and processing costs, FIG. 5B illustrates an improved process resulting from the combination of the first portion of the process described in FIG. 5A with the process of the present invention. It is clear from a comparison of the two schematic diagrams of FIG. 5 that the improved process requires fewer steps and is less complicated.

The process of FIG. 5B illustrates schematically the winning of nickel and associated metals from a sulfide ore by a hydrometallurgical process. As in FIG. 5A, the ore is first crushed and ground to a size appropriate for processing. Then a beneficiation operation is carried out, but with the difference that only the non-metal bearing portion of the ore is rejected. The concentrate produced contains a substantial portion of copper as well as nickel. A separate copper concentrate does not have to be processed by another means since the improved process of this invention can also separate copper from nickel with ease. After beneficiation, the metal concentrate is oxidatively leached with air and ammonia, as in the previous process. At this point, however, the leach solution is subjected to reaction with a carbon monoxide-containing gas and the metals are carbonylated. Separation of the various metal carbonyls is also accomplished and they are then easily recovered as the metals themselves.

Therefore, a preferred embodiment of this invention is a process for the recovery of nickel from a nickeliferous sulfide ore, said process comprising beneficiating the ore to produce a nickel-enriched concentrate thereof, oxidatively leaching the concentrate with an aqueous ammonia solution by injecting an oxygen-containing gas into a slurry of said concentrate, thereby dissolving the nickel values. The resultant leach solution is contacted with a carbon monoxide-containing gas under conditions whereby the nickel values are reduced to form nickel carbonyl. Nickel carbonyl is separated from the leach solution and decomposed to metallic nickel. As described previously, the contacting of the leach solution is preferably in the presence of a water-immiscible, substantially inert solvent for nickel carbonyl whereby the nickel carbonyl produced is concentrated in the solvent. Any of the solvents described previously may be used for dissolving the nickel carbonyl. However, a preferred solvent is a saturated aliphatic hydrocarbon. Another preferred process is characterized by carrying out the contacting of the leach solution in the presence of an amount of a promoter such as cyanide ion sufficient to catalyze the formation of nickel carbonyl. A preferred concentration of cyanide ion catalyst is from 0.01 to about 1 mole of cyanide ion per mole of nickel present. In lieu of the use of a solvent for nickel carbonyl, another preferred embodiment of this process is the separation of nickel carbonyl from the leach solution by passing a carbon monoxide-containing gas through the leach solution, allowing the nickel carbonyl to vaporize into the carbon monoxide-containing gas and subsequently passing the gas into a thermal decomposition zone wherein the nickel carbonyl is decomposed to metallic nickel.

In another preferred process, copper is recovered from the nickeliferous sulfide ore by a process similar to that represented in FIG. 5B. During the contacting of the leach solution with a carbon monoxide-containing gas, metallic copper is formed and deposits on the bottom of the reactor, or on granular copper added as nucleation sites. It should be recognized that this preferred process may also be characterized by the use of a cyanide ion catalyst and a water-immiscible solvent for nickel carbonyl. A preferred carbon monoxide-containing gas is selected from the group consisting of carbon monoxide and synthesis gas.

Cobalt is also recoverable by the process of this invention when the ore contains sufficient amounts thereof. A preferred process of this embodiment therefore includes the recovery of cobalt which is carbonylated in the leach solution forming cobalt tetracarbonyl anion. The cobalt is separated from the leach solution by injecting an oxygen-containing gas into the leach solution whereby cobalt tetracarbonyl anion is oxidized to hydrated cobalt oxide. The hydrated cobalt oxide is then heated to a temperature sufficient to drive off the waters of hydration to produce marketable cobalt oxide. Another preferred process of this invention includes the preparation of substantially pure metallic cobalt from cobalt oxide prepared in the above process by calcining the cobalt oxide in the presence of a reducing gas at a temperature sufficient to reduce cobalt oxide to substantially pure metallic cobalt.

Again it can be readily seen that the preferred process for producing cobalt and nickel may be further characterized by carrying out the contacting of the leach solution with a carbon monoxide-containing gas in the presence of cyanide ion catalyst and a water-immiscible solvent for nickel carbonyl.

From the above preferred process, one skilled in the art will readily understand that the process of this invention also includes the recovery of nickel, cobalt, and copper from a sulfide ore containing these materials according to the process represented schematically in FIG. 5B. Thus, a preferred process of this invention comprises beneficiating a nickeliferous sulfide ore containing recoverable amounts of copper and cobalt to produce a concentrate of said ore enriched in said nickel, copper, and cobalt, oxidatively leaching said concentrate with an aqueous ammonia solution by injecting an oxygen-containing gas into a slurry of a concentrate thereby dissolving the nickel, copper and cobalt values of the ore. The resultant leach solution is contacted with a carbon monoxide-containing gas under conditions whereby the nickel, copper, and cobalt values are reduced to form nickel carbonyl, metallic copper, and cobalt tetracarbonyl anion. The nickel carbonyl is separated from the leach solution and decomposed to metallic nickel. The copper metal is recovered from the leach solution as such. The cobalt is separated from the leach solution by injecting an oxygen-containing gas into the solution to oxidize cobalt tetracarbonyl anion to hydrated cobalt oxide. The hydrated cobalt oxide can then be heated at a temperature sufficient to drive off the waters of hydration to produce marketable cobalt oxide. The above process may be further characterized by the preferred embodiments of carrying out the contacting of the leach solution with a carbon monoxide-containing gas in the presence of a cyanide ion catalyst and a water-immiscible solvent for nickel carbonyl. In lieu of the water-immiscible solvent, nickel carbonyl may be recovered

in the above process by a carbon monoxide sweep as described previously.

The hydrometallurgical process for winning nickel from a sulfide ore described above as a preferred embodiment of this invention is illustrated by the following example.

#### EXAMPLE 26

A nickeliferous sulfide ore is screened, crushed, and ball-milled to obtain a final ore slurry of 90 percent minus 200-mesh. The slurry is separated in a wet drum-type magnetic separator. The non-magnetic pentlandite-chalcopyrite concentrate is sent to a classifier, and if necessary, reground in a ball mill to 85 percent minus 150-mesh. The ground product is conditioned in tanks by adding a water-soluble gum to depress flotation of talc in the gangue and tetra-sodium pyrophosphate as a dispersant. An amyl xanthate collector is also added in the conditioning tanks. The ore is floated in a roughing circuit from which a bulk nickel-copper concentrate is removed. The underflow goes to a scavenging section to remove additional nickel-copper and iron; this product is again fed to magnetic separators and goes through the flotation scheme after removal of any remaining pyrrhotite.

The pentlandite-chalcopyrite is fed to an autoclave and leached with air and ammonia under about 120 psig. and at 180°F. The leach solution is thickened by continuous counter-current decantation and the leach liquor sent to recover the copper, nickel and cobalt. The thickened residual slurry is filtered, pulped with aqueous ammonia, and again leached with air and ammonia. The slurry from the second stage leaching is thickened, filtered and washed and the filtrate is recycled to the first stage leach. The residue from the second stage leach is slurried and sent to impounding basins.

The leach liquor from the first stage leach is added with potassium cyanide and kerosene to a pressure autoclave. The autoclave is pressured to about 600 psig. with synthesis gas at 250°F. and stirred mechanically. As the pressure decreases, additional synthesis gas is added to maintain a pressure of about 600 psig. After three hours, the reaction autoclave is cooled and vented. The hydrocarbon phase is decanted and sent for nickel recovery. The aqueous phase is sent to cobalt recovery. Copper metal is removed from the autoclave.

The kerosene-containing nickel carbonyl is distilled to recover the nickel carbonyl which is then decomposed to metallic nickel. A good yield of nickel is obtained.

Similar results may be obtained by using HCN instead of potassium cyanide. Also, the kerosene is not necessary and the nickel carbonyl formed may be vented directly to the thermal decomposition zone. Additional synthesis gas is used to sweep out the reaction autoclave, thus recovering all of the nickel carbonyl produced.

Additional variations will be apparent to a skilled practitioner in the art without departing from the scope of this process. It is clear that the process of this invention has the advantages of reduced milling and processing steps with a resultant saving in capital investment and processing costs.

Another preferred embodiment of this invention is illustrated by FIG. 6. FIG. 6A schematically describes a process known in the art for winning nickel by flash smelting a nickel concentrate, converting the nickel-

iron matte to a nickel sulfide matte, removing copper by a two-stage leaching step, then precipitating cobalt by reacting with "black" nickel hydroxide and subjecting the nickel produced to electro-winning to produce pure nickel cathodes.

The flash smelting technique combines a roasting and smelting procedure into one operation requiring no external fuel. The sulfur and iron content of the ore concentrate burn with preheated air to roast and smelt the ore. Finely divided ore concentrate is added to the furnace with a flux material, usually quartz sand, and oxygen or air preheated to about 900°F. While in suspension, the sulfur and iron "combine" with oxygen in a "flash" combustion producing smelting temperatures. The usual smelting and slagging reactions occur and a nickel-iron matte is produced. The grade of matte depends on the ratio of oxygen to sulfur in the feed. Two types of flash smelters have been developed. One is a rectangular reverberatory-type with burners at both ends and a central gas uptake. The other is an upright U-shaped furnace with a vertical reaction shaft at one end down which the flashing occurs, a horizontal reverberatory settler and a vertical gas uptake at the other end through which combustion gases exit. Typical analysis of one flash smelted matte is 35 percent nickel, 12 percent copper, 25 percent iron, and 24 percent sulfur. The content of course depends on the ore, the amount of beneficiation, and the ratio of air to sulfur in the flash smelting operation.

The matte is then converted by blowing with air to remove the iron and reduce the sulfur. Additional flux material, again usually quartz sand, is added to facilitate slagging. The converter matte typically produced analyzes 63 percent nickel, 28 percent copper, and 7 percent sulfur.

Nickel can be recovered from the slag by electric furnace smelting with coke and recycled scrap. The electric furnace matte can then be added to the converter charge.

The nickel sulfide matte from the converter is granulated by pouring the molten matte into water. Usually on cooling, sufficient sulfur is available only to combine with the copper as copper sulfide,  $Cu_2S$ . Any extra sulfur combines with nickel as nickel sulfide,  $Ni_3S_2$ .

The granulated matte is then crushed and ground and leached with ammonia in a two-stage operation to remove copper. The first stage consists of repulping the ground matte with decopperized solution containing free acid and adding barium carbonate,  $BaCO_3$ . The pulp is pumped to leaching tanks where mechanical agitation with air causes nickel to dissolve. Copper cements out and is redissolved as copper sulfate. The lead reacts with barium carbonate to form lead sulfate. Any iron in the solution precipitates as ferric hydroxide. These are removed by cyclone and counter-current decantation thickener in series. The pregnant solution overflowing the thickener still containing cobalt is filtered and reacted with "black" nickel hydroxide to remove cobalt. Black nickel hydroxide is prepared electrolytically by oxidizing nickel hydroxide under conditions that produce tetravalent as well as trivalent nickel hydrates. The cobalt precipitates as cobalt hydroxide in air agitated tanks. The solution containing nickel hydroxide is then filtered, preheated and then sent to an electro-winning tank to produce nickel cathodes containing 99.95 percent nickel.

FIG. 6B schematically represents an improved pro-

cess which includes, after the usual crushing and grinding, beneficiating, flash smelting, and converting, oxidatively leaching to dissolve the nickel values, followed by carbonylation under conditions whereby nickel carbonyl is produced, and separation from the reaction medium. The nickel values in the form of nickel carbonyl are then recovered.

Therefore, a preferred embodiment of this process is a process for recovering nickel from a nickeliferous sulfide ore, said process comprising beneficiating the ore to produce a concentrate thereof enriched in nickel, mixing the concentrate with quartz sand, and smelting the mixture to produce a matte containing nickel, iron, and sulfur, oxidatively leaching the matte with an aqueous ammoniacal ammonium salt solution by injecting an oxygen-containing gas into a slurry of the matte, thereby dissolving the nickel values in the ore. The resultant leach solution is contacted with a carbon monoxide-containing gas under conditions whereby the nickel values are reduced to form nickel carbonyl. The nickel carbonyl is then separated from the leach solution and decomposed to metallic nickel. As previously described, the contacting of the leach solution with a carbon monoxide-containing gas is preferably carried out in the presence of an essentially water-immiscible, substantially inert solvent for nickel carbonyl whereby the nickel carbonyl is concentrated in the solvent. Any of the previously described solvents may be used in the preferred process. A most preferred solvent is a saturated aliphatic hydrocarbon.

Also, the process may be further characterized by carrying out the contacting in the presence of an amount of cyanide ion sufficient to catalyze the formation of nickel carbonyl. A preferred concentration of cyanide ion catalyst is from 0.01 to about 1 mole of cyanide ion per mole of nickel present.

The aqueous ammoniacal ammonium salt solution is preferably selected from the group consisting of aqueous ammoniacal ammonium chloride, carbonate, sulfate, or mixtures thereof. Also, aqueous ammonium hydroxide can be employed as the leaching media. A most preferred aqueous ammoniacal ammonium salt solution is aqueous ammoniacal ammonium carbonate. The oxidative leach is preferably carried out with an oxygen-containing gas selected from the group consisting of oxygen-enriched air and oxygen. A most preferred oxygen-containing gas is oxygen.

In lieu of the use of a solvent for nickel carbonyl, the nickel carbonyl can be separated from the leach solution by passing a carbon monoxide-containing gas through the leach solution, allowing the nickel carbonyl to vaporize into the carbon monoxide-containing gas, and subsequently passing the carbon monoxide-containing gas into a thermal decomposition zone wherein the nickel carbonyl is thermally decomposed to metallic nickel.

One skilled in the metal art will readily recognize that the preferred process of this embodiment is also amenable to recovering copper and cobalt. Thus, it is a most preferred process of this embodiment to recover nickel, copper, and cobalt by a process comprising beneficiating an ore containing recoverable amounts of nickel, copper, and cobalt to produce a concentrate enriched in nickel, copper, and cobalt, mixing the concentrate with quartz sand, and smelting the mixture to produce a matte containing nickel, copper, cobalt, iron, and sulfur, oxidatively leaching the matte with an

aqueous ammoniacal ammonium salt solution such as ammoniacal ammonium carbonate or sulfate by injecting an oxygen-containing gas into a slurry of the matte, thereby dissolving the nickel, copper, and cobalt values. The resultant leach solution is then contacted with a carbon monoxide-containing gas under conditions whereby the nickel, copper, and cobalt values are reduced to form nickel carbonyl, metallic copper and cobalt tetracarbonyl anion. The nickel carbonyl is then separated from the leach solution and decomposed to metallic nickel. The metallic copper can then be recovered from the leach solution. The cobalt is separated from the leach solution by injecting an oxygen-containing gas into the leach solution whereby the cobalt tetracarbonyl anion is oxidized to hydrated cobalt oxide. The hydrated cobalt oxide is then heated to drive off the waters of hydration to produce marketable cobalt oxide. As described above, most preferred processes for recovery of nickel, copper, and cobalt include the use of an aqueous ammoniacal ammonium salt solution selected from aqueous ammoniacal ammonium chloride, carbonate, sulfate, or mixtures thereof. Also, aqueous ammonium hydroxide may be employed in this process. Further, most preferred processes of this invention are characterized by carrying out the contacting with the carbon monoxide-containing gas in the presence of cyanide ion catalyst and a water-immiscible solvent for nickel carbonyl. As previously described, the nickel carbonyl can be separated from the leach solution by utilizing a carbon monoxide sweep instead of by extracting into a solvent for nickel carbonyl.

In addition to the above preferred embodiment, it is also possible to recover nickel by this process using a converting step to eliminate iron and decrease the sulfur content of the matte to form a substantially iron-free, low sulfur nickel matte. Thus, it is a preferred process of this invention to recover nickel from a nickeliferous sulfide ore by a process comprising beneficiating the ore to produce a concentrate enriched in nickel, mixing the concentrate with quartz sand and smelting the mixture to produce a matte containing nickel, iron, and sulfur, and then mixing the nickel-iron-sulfur matte with additional quartz sand and converting the mixture by blowing with air at elevated temperature forming a substantially iron-free, low sulfur, nickel matte. This matte is then oxidatively leached and contacted with a carbon monoxide-containing gas as described previously to produce nickel carbonyl which may be decomposed to metallic nickel.

Most preferred processes of this invention utilize the presence of an essentially water-immiscible, substantially inert solvent, preferably a saturated aliphatic hydrocarbon, and a catalytic amount of cyanide ion, preferably from 0.01 to about 1 mole of cyanide ion per mole of nickel present. Again, as previously described, a preferred process may employ a carbon monoxide sweep to separate the nickel carbonyl from the leach solution instead of a solvent for nickel carbonyl. It should be further recognized that copper and cobalt may be recovered from an ore containing recoverable amounts thereof by the process of this invention.

This preferred embodiment is further illustrated by reference to the following example.

#### EXAMPLE 27

A nickeliferous sulfide ore is comminuted by crushing and grinding and then screened until 90 percent of

the ore passes a 200-mesh screen. The ore is beneficiated by flotation to produce a pentlandite-pyrrhotite concentrate containing 6 percent nickel and 0.5 percent copper. The ore is dried in a rotary kiln and charged to a flash smelter with quartz sand and pre-heated air at 900°F. The smelter produces a matte having a typical analysis as follows:

35% nickel

12% copper

25% iron

24% sulfur

The matte is charged to a converter with quartz sand and blown with air to produce a substantially iron-free matte containing typically:

15 63% nickel

28% copper

7% sulfur

0.4% iron

The matte is granulated by pouring the molten converter product through a water spray and into quench tanks containing an ammoniacal ammonium carbonate solution. The slurry is then fed to aerating units in which air is injected dissolving the nickel, copper, and cobalt. The leach solution is separated from the slurry

25 by a series of counter-current decantation thickeners. The residual slurry is washed and thickened to recover nickel, copper and cobalt values and the overflow added to the pregnant leach solution. The leach solution is placed in a pressure reaction vessel with a catalytic amount of 1 M KCN. The reactor is sealed, flushed with carbon monoxide, and pressured to 300 psig. The temperature is brought to 250°F. and mechanical agitation is initiated. Additional carbon monoxide is pressured into the reactor as the pressure de-

30 creases because of carbon monoxide uptake in the formation of nickel carbonyl. After 2 hours, the pressure does not decrease and the reaction is complete. The reactor is cooled and the nickel carbonyl and unreacted carbon monoxide are vented to traps containing bromine where the nickel carbonyl reacts to form  $\text{NiBr}_2$ .

35 The cobalt tetracarbonyl anion is recovered from the leach solution and copper metal deposited on the bottom of the reaction vessel is collected. All metal values are recovered in good yield.

40 45 Similar results may be obtained when the reaction with carbon monoxide is carried out in the presence of a water-immiscible, substantially inert solvent for nickel carbonyl, for example, an aliphatic hydrocarbon such as heptane. Also similar results are obtained when the nickel carbonyl is vented to a thermal decomposition zone by sweeping out the reaction autoclave with carbon monoxide and decomposing nickel carbonyl to metallic nickel. Similar results are obtained when the carbon monoxide is replaced with synthesis gas.

50 55 From a converter matte having the following analysis:

64.5% nickel

25.7% copper

6.1% sulfur

0.38 % cobalt

0.63% iron

0.15% arsenic

0.2% silicon

60 65 trace — Other elements

an oxidative leach and reductive carbonylation was run. The procedure followed was to crush and grind the granulated matte in a ball mill to less than 100-mesh. The ground matte was then placed in an autoclave fit-

ted with thermocouples, heating means, stirring means, pressure gauges, gas inlet and vent lines. Then the autoclave was charged with aqueous ammonia and ammonium carbonate or sulfate, plus enough water to make a suitable reaction volume. The vessel was then sealed and pressured with oxygen or air and heated to 176°F. After reaction, the reactor contents were filtered and the solution was analyzed for nickel and copper. The following Table III summarizes the results of the oxidative leach step.

TABLE III.—OXIDATIVE LEACH OF SULFIDE MATTE

| Example No. | NH <sub>4</sub> <sup>+</sup>       |                               | H <sub>2</sub> O, g. | Oxidizing agent    | Pressure uptake, p.s.i. | Temp., °C. | Time, min. | Percent dissolved |       |
|-------------|------------------------------------|-------------------------------|----------------------|--------------------|-------------------------|------------|------------|-------------------|-------|
|             | NH <sub>4</sub> OH, 30% conc., ml. | Anion                         |                      |                    |                         |            |            | Ni                | Cu    |
| 28          | 60                                 | SO <sub>4</sub> <sup>2-</sup> | 17.5                 | 60 O <sub>2</sub>  | 218                     | 80         | 157        | 92                | 92    |
| 29          | 30                                 | SO <sub>4</sub> <sup>2-</sup> | 8.8                  | 30 Air             | 1200                    | 80         | 360        | 96                | 94    |
| 30          | 2.5                                | CO <sub>3</sub> <sup>2-</sup> | 14                   | 100 O <sub>2</sub> | 79                      | 80         | 196        | 73.4              | 61.5  |
| 31          | 60                                 | CO <sub>3</sub> <sup>2-</sup> | 14                   | 40 O <sub>2</sub>  | 224                     | 80         | 231        | 106               | 99    |
| 32          | 2                                  | CO <sub>3</sub> <sup>2-</sup> | 4                    | 48 O <sub>2</sub>  | (2)                     | R.T.       | 120        | 99                | 79.6  |
| 33          | 2                                  | CO <sub>3</sub> <sup>2-</sup> | 2                    | 48 Air             | (2)                     | R.T.       | 188        | 96.8              | ----- |

<sup>1</sup> A few minutes after pressuring to 100 p.s.i. with air, the pressure dropped to 80 p.s.i. The remaining nitrogen was vented to 0 p.s.i. and the reactor repressured to 100 p.s.i. with air. This was done ten times before the decrease in pressure stopped above 80 p.s.i.

<sup>2</sup> In this run the leach was carried out at atmospheric pressure. The oxidizing agent is bubbled through the solution at 0.006 cubic feet per minute. Periodically the reaction was stopped and samples taken to check the progress of the reaction.

## EXAMPLE 34

Using the product of Example 28, 100 ml. of the leach solution was charged to a 300 ml. stainless steel autoclave with 1.0 ml. of 1 M KCN. The reactor was flushed with carbon monoxide and pressured to 50 psig. After heating to 125°C. the pressure was increased to 300 psig. and stirring initiated. After 30 minutes with slow pressure decrease, the temperature was raised to 150°C. and the carbon monoxide pressure increased to 400 psig. The total reaction time was 147 minutes and total carbon monoxide pressure uptake was 159 psig. The reactor was cooled to 50°C. and vented into a series of two bromine traps and an olefin trap. The reactor autoclave was repressured with carbon monoxide to 300 psig. three times and vented to the traps, removing all of the nickel carbonyl formed. The bromine trap solutions were treated with olefins to remove unreacted bromine and the NiBr<sub>2</sub> was extracted with water. The NiBr<sub>2</sub> solution was analyzed and found to produce a 95 percent recovery of nickel as nickel carbonyl from the leach solution.

The aqueous solution in the reactor was heated to 140°F. for a few minutes and filtered. The solids analyzed 97 percent copper and 3 percent nickel. The filtrate was analyzed and showed 33 percent of the copper charged to the leach solution was recovered. The combined recovery of copper from the leach solution was 83 percent.

A still further preferred embodiment of the improved process for winning nickel is schematically illustrated in FIG. 7. This process for winning nickel, illustrated in FIG. 7A, provides for crushing and grinding a sulfide ore, beneficiating the ore to produce a nickel concentrate. The concentrate is charged to a vertical rotary converter with a top-blown oxygen lance and a nickel-iron matte is produced. The matte is drastically quenched to produce granules of matte containing a solid "active" nickel product which is then subjected to carbonylation under high temperatures and pressures. A complicated scheme for separating nickel values and recovering other metal values after the carbonylation includes separation of iron and nickel carbonyls from

the solid residues. The iron and nickel carbonyls are then decomposed to produce a ferro-nickel product, or a further separation produces nickel carbonyl which is decomposed to nickel metal. The solid residues are leached under pressure to produce a copper-containing solution from which copper may be produced in an electrowinning process, and a nickel-cobalt-iron solution which is purified to produce cobalt powder and nickel carbonate, the iron being sent to waste. A third process stream from the pressure leach step subjects

25 the solid residues to sulfur removal and a second leach operation. The copper removed is combined with that produced from the first leach and sent to electrowinning. The residues from the second leach are smelted and sent for recovery of the precious metals contained 30 therein. This process is more fully described in Canadian Pat. No. 822,616, issued Sept. 2, 1969.

The process of FIG. 7B represents an improvement in that metal values are obtained in a more useful form and with substantial saving in capital investment and 35 processing costs. The schematic diagram of FIG. 7B represents a preferred embodiment of this invention for winning metals from a sulfide ore. The process includes, as usual, crushing and grinding the ore, beneficiating it to produce a nickel concentrate, smelting the 40 ore in a vertical rotary converter with a top-blown oxygen lance, and drastically quenching the nickel-iron matte produced to obtain the "active" nickel product in granule form. The improvement is to then leach the granules with an ammonium salt solution to produce a 45 nickel-containing solution which can be carbonylated at lower temperatures and pressures than is true of the process of FIG. 7A. In addition, metals associated with nickel such as copper and cobalt are treated in the same operation and carbonyl compounds of copper and cobalt are produced thereby. These are separated 50 from the reaction mixture and the metal values recovered.

Therefore, a preferred embodiment of this invention 55 is a process for recovering nickel from a nickeliferous sulfide ore, said process comprising beneficiating said ore to obtain a concentrate enriched in nickel, mixing said concentrate with a siliceous flux, and converting the mixture at a temperature sufficient to maintain at least part of the concentrate in a molten state by blowing the melt with air or oxygen-enriched air through a lance directed at the upper surface of the melt in a top-blown rotary converter to produce a low-sulfur metal melt. The melt is then drastically quenched whereby a fine-grained granular nickel product is produced. The granular nickel product is then oxidatively leached with an aqueous ammoniacal ammonium salt solution by injecting an oxygen-containing gas into a slurry of the 60 65

granular nickel product, thereby dissolving the nickel values. The resultant leach solution is contacted with a carbon monoxide-containing gas under conditions whereby the nickel values are reduced to form nickel carbonyl. The nickel carbonyl is separated from the leach solution and decomposed to metallic nickel.

As previously described, it is a preferred embodiment of the above process to carry out the contacting with a carbon monoxide-containing gas in the presence of an essentially water-immiscible, substantially inert solvent for nickel carbonyl whereby the nickel carbonyl produced is concentrated in the solvent. A preferred solvent is saturated aliphatic hydrocarbon.

Another preferred process of this invention is characterized by carrying out the contacting with a carbon monoxide-containing gas in the presence of an amount of cyanide ion sufficient to catalyze the formation of nickel carbonyl. A most preferred amount of cyanide ion catalyst is from about 0.01 to about 1 mole of cyanide ion per mole of nickel present.

In lieu of separating the nickel carbonyl from the leach solution with a water-immiscible solvent, it is a preferred embodiment of the above process to recover nickel carbonyl from the leach solution by passing a carbon monoxide-containing gas through the leach solution, allowing the nickel carbonyl to vaporize into the carbon monoxide-containing gas and subsequently passing it into a thermal decomposition zone wherein nickel carbonyl is decomposed to metallic nickel.

A preferred aqueous ammoniacal ammonium salt solution for carrying out the oxidative leach is selected from the group consisting of aqueous ammoniacal ammonium chloride, carbonate, sulfate, or mixtures thereof. Another leaching media is aqueous ammonium hydroxide. A most preferred aqueous ammoniacal ammonium salt solution is aqueous ammoniacal ammonium carbonate. The oxidative leach may be further characterized by carrying out the leach with an oxygen-containing gas selected from the group consisting of oxygen-enriched air and oxygen. A most preferred oxygen-containing gas is oxygen.

It should be recognized that this process is amenable to recovery of copper and cobalt as well as nickel values. Thus, it is a preferred process of this embodiment to recover nickel, copper, and cobalt when the ore contains recoverable amounts of these materials by a process comprising beneficiating the ore to obtain a concentrate enriched in nickel, copper, and cobalt, mixing the concentrate with a siliceous flux, and converting the mixture at a temperature sufficient to maintain at least part of said concentrate in a molten state by blowing the melt with air or oxygen-enriched air through a lance directed at the upper surface of said melt in a top-blown rotary converter to produce a low-sulfur metal melt. The melt is then drastically quenched whereby a finely grained, granular product containing nickel, copper and cobalt is produced. The granular nickel product is oxidatively leached with aqueous ammoniacal ammonium salt solution by injecting an oxygen-containing gas into a slurry of the granular nickel product, thereby dissolving the nickel, copper and cobalt values. The resultant leach solution is contacted with a carbon monoxide-containing gas under conditions whereby the nickel, copper and cobalt values are reduced to form nickel carbonyl, metallic copper, cobalt tetracarbonyl anion. The nickel carbonyl is separated from the leach solution and decomposed to metallic

nickel. Metallic copper is then recovered from the leach solution. Cobalt is separated from the leach solution by injecting an oxygen-containing gas into the leach solution whereby cobalt tetracarbonyl anion is oxidized to hydrated cobalt oxide and the hydrated cobalt oxide is heated at a temperature sufficient to drive off the waters of hydration to produce cobalt oxide.

As previously described, the aqueous ammoniacal ammonium salt solution is preferably selected from the 10 group consisting of aqueous ammoniacal ammonium chloride, carbonate, and sulfate. Also, preferred embodiments of the above process for winning and separating nickel, copper, and cobalt may be further characterized by the use of one of the previously-described 15 promoters such as a cyanide ion catalyst. Also, a water-immiscible, substantially inert solvent for nickel carbonyl can be used. However, in lieu of the water-immiscible solvent, nickel carbonyl may preferably be separated from the leach solution by using a carbon 20 monoxide sweep and thermal decomposition of nickel carbonyl to metallic nickel as more fully described hereinabove.

The preferred embodiment of this invention is further illustrated by the following example. The feed material is a combination of the metallic fraction of a matte separation process, a copper-nickel alloy containing precious metals, residues from electrolytic refining of nickel sulfide anodes, and crude nickel sulfide concentrates. These materials are subjected to the 25 usual crushing and grinding, and then briquetted or pelletized to form a charge of uniform composition as described below.

#### EXAMPLE 35

35 A feed consisting of briquettes and pellets of nickel-containing materials has the following typical analysis:

|     |        |
|-----|--------|
| 62% | nickel |
| 14% | copper |
| 1%  | cobalt |
| 2%  | iron   |
| 20% | sulfur |

40 The feed is charged to a vertical rotary top-blown converter. The feed is melted with an oxy-fuel lance and brought to about 2,500°F. While the converter rotates to induce mechanical agitation, the melt is then top-blown with oxygen until the sulfur content is decreased to a desirable level—usually about 4,290°. The melt 45 temperature is increased to about 2900°F. by the blowing. The molten product is poured from the converter into a holding furnace and from there is poured through a water spray to drastically quench and granulate the molten converter product. The granules thus 50 prepared are fine-grained solid solution having the same composition as the molten converter melt.

55 The granules are then slurried with aqueous ammoniacal ammonium carbonate and the slurry is fed into aerating units. The nickel, cobalt, and copper values are dissolved and the pregnant solution is separated by a series of counter-current decantation thickeners. The 60 underflow from the thickeners is washed to recover nickel, copper, and cobalt values and the residue sent to recover the precious metals.

The pregnant solution is fed into a pressure autoclave 65 with potassium cyanide added as a catalyst. The autoclave is pressured with carbon monoxide to 300 psig. and heated to 250°F. while the reaction solution is mechanically agitated. After three hours, the autoclave

contents are cooled and the pressure released into a vent line which leads to a thermal decomposition zone. The nickel carbonyl formed in the reaction is decomposed to metallic nickel. To insure recovery of all the nickel as nickel carbonyl from the reactor, carbon monoxide is passed through the autoclave to volatilize and sweep out any product nickel carbonyl to the decomposition zone. The nickel carbonyl is heated rapidly to about 400°F. to produce carbon monoxide and metallic nickel. A good yield is obtained.

The copper in the solution fed to the reaction autoclave is reduced to metallic copper and can be recovered in good yield as such from the vessel.

The cobalt is carbonylated to cobalt tetracarbonyl anion and remains in the reaction solution. It can readily be separated by injecting oxygen into the solution to produce hydrated cobalt oxide which is filtered off. On heating the filter cake, the waters of hydration are vaporized and cobalt oxide is recovered in good yield.

The skilled practitioner will readily appreciate the variations which may be employed in this preferred embodiment by incorporating other preferred conditions and procedures hereinabove described.

A still further preferred embodiment is illustrated by FIG. 8. The schematic process flow diagram in FIG. 8A represents a process for winning nickel values from a nickel-containing sulfide ore. The process shown includes the usual ore preparation steps of crushing, grinding, and beneficiation to produce a nickel concentrate. Also, copper and iron concentrates are produced which are further processed. The nickel concentrate is roasted, smelted and converted to produce a nickel-sulfide matte. The matte is then allowed to cool very slowly over a period of days. This slow cooling allows the formation of discrete crystals of metals and metal sulfides. The solid matte is again crushed, ground, and beneficiated to obtain a nickel concentrate which is again roasted. A nickel oxide product is obtained. The residue may be either smelted with coke to produce a nickel sulfide matte which is cast into anodes for electrowinning of pure nickel or reduced and subjected to carbonylation according to the Mond process with subsequent decomposition to nickel metal.

The ore is subjected to the usual crushing, grinding and beneficiation as previously described. The nickel concentrate is then subjected to a roast with the addition of a siliceous flux in a multi-hearth roaster. The roaster using oxygen-enriched air is charged with about 25-30 wt. % of the flux. The concentrate containing about 6 percent nickel-copper, 42 percent iron, 28 percent sulfur, and 12 percent moisture is roasted at about 700° to 1,500°F. The roasting decreases the sulfur content to about 12.5 percent and the final calcine discharged from the roaster is charged to conveyors which carry the calcine to the reverberatory furnace for smelting.

The smelting in this process is carried out in a reverberatory furnace which has the advantage of being able to smelt material of fine particle size, for example, flotation concentrates, without blowing it from the furnace. Reverberatory furnaces are long rectangular structures with an arched roof and burners at one end and the exhaust gas flue at the other end. The charge is fed through fettling pipes in the roof arranged along the sides into the interior of the furnace. Fuel, such as pulverized coal, oil, or natural gas, is burned above the charge with the flame extending about half the length

of the furnace. The charge along the sides is melted from direct heat of the flame and from heat radiating from the roof and sides of the furnace. As the charge melts, it flows toward the center of the furnace with the matte and slag separating. The combustion generates temperatures of about 3,000°F. at the burner end. The temperature falls off to about 2,400°F. at the gas exit, but is sufficiently hot to maintain the slag and matte in a molten state. Slag and matte are tapped after sufficient time for the smelting reactions to occur and the gravity settling to separate the slag from the matte.

The matte, typically containing about 15 percent nickel-copper, is fed to horizontal side blown converters and with siliceous flux is blown to a low-iron, sulfur deficient matte. the use of oxygen-enriched air improves blowing efficiency and decreased loss of heat via inert nitrogen. The converter matte typically analyzes:

47nickel

20 30% copper  
0.5% iron  
22% sulfur

In addition, small amounts of gold, silver, and platinum and other impurities are present. The converter slag 25 containing 2.3 percent nickel-copper is returned to the reverberatory furnace to recover the nickel and copper.

The nickel-copper matte is poured into special cooling molds which allows the matte to cool slowly over a period of 3 days from about 1,800°F. to about 900°F.

30 The mold covers are then removed and further cooling to about 400°F. is allowed for another day. This slow cooling process permits phase separation and promotes larger grain size. On cooling, the matte separates into discrete copper sulfide, nickel sulfide, and metallic nickel-copper alloy. The slow cooling in particular permits the different materials to solidify separately and allows diffusion of the still liquid phases from the solidifying material. For example, at 1,690°F. solid copper

35 sulfide crystals begin to form. As cooling continues, more solid copper sulfide forms and the remaining liquid phase is enriched in nickel. The slow cooling promotes the formation of coarse grains. At about 40,1,290°F. a metallic nickel-copper alloy begins to solidify.

45 As cooling continues further, the nickel sulfide begins to solidify at 1,067°F. As the matte cools from this point, a structural transformation of nickel sulfide occurs in which the form of nickel sulfide has a lowered solubility for copper sulfide and metallic phases. Thus, 50 the nickel sulfide rejects additional amounts of the copper sulfide and metallic phase and typically has less than 0.5 percent copper below about 700°F. The cooled matte is then a solid ingot containing coarse grained particles of the three phases — copper sulfide, nickel sulfide, and metallic nickel-copper alloy.

55 The ingot is lifted from the mold, broken into chunks and crushed and ground. The grinding fractures the ingot at the boundaries of the grains and not through the grains themselves. Thus, the copper sulfide, nickel sulfide, and metallic phases are liberated. They are then separated by beneficiation similar to that used in the ore preparation. The copper sulfide concentrate produced is sent to copper smelters and the metallic nickel-copper alloy after cleaning is recycled to the smelter.

60 The nickel sulfide is either melted and cast into anodes for electro-refining or roasted. For the roasting, a

fluid bed reactor is used. The nickel sulfide concentrate with 10 percent by weight of the dust recovered from the roaster is pulped in water and fed via a constant head tank to internal drum filters. The filter cake is then pelletized on a rotating disk to about  $\frac{1}{4}$ -inch diameter pellets. Pelletizing is necessary to prevent the fine nickel sulfide particles obtained from the flotation concentrate from softening and sticking which occurs at about 200°F. at normal sulfur removal temperatures which is much higher than 1,200°F. Roasting temperatures of about 1,800°F. are required to remove sulfur from nickel sulfide and produce a low-sulfur calcine. Also, the fluid bed operation is more amenable to a feed material which is not too fine. The pellets are an excellent feed material and allow satisfactory fluidization, are sufficiently large to not soften quickly on heating to about 2,000°F. Space velocities in the fluidized beds are generally about 7. The roasting is done with 20 to 30 percent by volume of air above the stoichiometric requirements for combining with the nickel. The roast causes reaction of nickel sulfide and oxygen to form nickel oxide and sulfur dioxide. The nickel oxide is discharged from the roaster as a calcine containing about 0.2 percent by weight sulfur.

The calcine is cooled in fluidized bed coolers into which water is sprayed at the top and air enters at the bottom. The calcine is quickly quenched from 2,000°F. to about 200°F. Further processing operations which combine with the roast are electrolytic refining and carbonylation by the Mond Process. Another avenue of approach is to deep roast the calcine at higher temperatures of about 2,250°F., using oxygen-enriched air. A nickel oxide product having 0.05 percent sulfur is produced. Further roasting of this low-sulfur nickel oxide with chlorine reduces the copper to about 0.25 percent by weight. A hydrogen reduction step removes about 75 percent of the oxygen to produce nickel product which is 90 percent by weight nickel.

A comparison of the process of FIG. 8A with the preferred process of this invention schematically represented in FIG. 8B shown an obvious advantage in fewer processing steps with resultant saving in capital investment and processing costs. The process represented by FIG. 8B contains the crushing and grinding, beneficiation, roasting, smelting and converting steps of the previous process. However, the improvement lies in oxidatively leaching the converter matte and then carbonylating the leach solution under reducing conditions to produce carbonyl compounds of nickel and its associated metals, for example, copper and cobalt. These are separated and recovered as the metals.

Thus, it is a preferred embodiment of this invention to recover nickel from nickeliferous sulfide ore by a process comprising:

- a. beneficiating said ore to produce a concentrate enriched in nickel,
- b. roasting the concentrate with a siliceous flux in the presence of air or oxygen-enriched air to produce a calcine having a reduced sulfur content,
- c. smelting the calcine to produce a nickel-iron matte,
- d. converting the nickel-iron matte by blowing with air or oxygen-enriched air at a temperature sufficient to maintain at least part of said matte in the molten state substantially reducing the sulfur and iron content of the matte,

- e. oxidatively leaching the converted matte with an aqueous ammoniacal ammonium salt solution by injecting an oxygen-containing gas into a slurry of the converted matte in said aqueous ammoniacal ammonium salt solution thereby dissolving the nickel values in the converted matte,
- f. contacting the resultant leached solution with a carbon monoxide containing gas under conditions whereby the nickel values are reduced to form nickel carbonyl,
- g. separating the nickel carbonyl from the leached solution, and
- h. decomposing the nickel carbonyl to metallic nickel.
- 15 A further preferred embodiment of the above process is a process wherein the contacting of Step (f) is carried out in the presence of an essentially water immiscible, substantially inert solvent for nickel carbonyl whereby said nickel carbonyl is concentrated in the solvent.
- 20 Any of the previously-described solvents is suitable for this preferred embodiment. A most preferred solvent is a saturated aliphatic hydrocarbon. Another preferred process is characterized by carrying out the contacting of step (f) in the presence of one of the
- 25 previously-described promoters such as an amount of cyanide ion sufficient to catalyze the formation of nickel carbonyl. A most preferred amount of cyanide ion is from 0.01 to about 10 moles of cyanide ion per mole of nickel.
- 30 In lieu of the water-immiscible solvent, it is a preferred process of this invention to separate nickel carbonyl from the leach solution in step (g) above, by passing a carbon monoxide-containing gas through the leach solution allowing nickel carbonyl to vaporize into the carbon monoxide-containing gas and subsequently decomposing the nickel carbonyl by passing the carbon monoxide-containing gas into a thermal decomposition zone wherein nickel carbonyl is decomposed to metallic nickel.
- 35
- 40 In a further preferred process the aqueous ammoniacal ammonium salt solution in step (e) above is selected from the group consisting of aqueous ammoniacal ammonium chloride, carbonate, sulfate, or mixtures thereof. Also, aqueous ammonium hydroxide may preferably be employed. A most preferred aqueous ammoniacal ammonium salt solution is aqueous ammoniacal ammonium carbonate.
- 45 Another preferred embodiment of the above process is further characterized by carrying out the oxidative leach of step (3) above with an oxygen-containing gas selected from the group consisting of oxygen-enriched air and oxygen.
- 50 One skilled in the art will appreciate that this process is suitable for recovery and separation of recoverable amounts of nickel, copper and cobalt. Therefore, it is a preferred embodiment of the above process for recovering nickel to recover copper and cobalt by a similar process comprising:
- 55
- 60 a. beneficiating the ore to produce a concentrate enriched in nickel, copper and cobalt;
- b. roasting the concentrate with a siliceous flux in the presence of oxygen or oxygen-enriched air to produce a calcine having a reduced sulfur content;
- c. smelting said calcine to produce a matte containing nickel, copper, cobalt, iron and sulfur;
- d. converting the matte by blowing with air or oxygen-enriched air at a temperature sufficient to

- maintain at least part of the matte in the molten state, substantially reducing the amount of sulfur and iron content of the matte;
- e. oxidatively leaching the converted matte with an aqueous ammoniacal ammonium salt solution by injecting an oxygen-containing gas into a slurry of the converted matte in said aqueous ammoniacal ammonium salt solution, thereby dissolving the nickel, copper and cobalt values in the converted matte;
  - f. contacting the resultant leach solution with a carbon monoxide-containing gas under conditions whereby the nickel, copper and cobalt values are reduced to form nickel carbonyl, metallic copper and cobalt tetracarbonyl anion;
  - g. separating the nickel carbonyl from the leach solution;
  - h. decomposing nickel carbonyl to metallic nickel;
  - i. recovering the metallic copper from the leach solution;
  - j. separating the cobalt from the leach solution by injecting an oxygen-containing gas into the leach solution whereby the cobalt tetracarbonyl anion is oxidized to hydrated cobalt oxide; and
  - k. heating the hydrated cobalt oxide at a temperature sufficient to drive off the waters of hydration to produce cobalt oxide.

One skilled in the art will appreciate from the above description that this preferred process may be carried out using an aqueous ammoniacal ammonium chloride, carbonate, or sulfate solution, or mixtures thereof. Also, aqueous ammonium hydroxide may be used as the leach solution. The above process may be further characterized by carrying out the contacting in step (f) in the presence of an amount of cyanide ion sufficient to catalyze the formation of nickel carbonyl. Further, step (f) may be carried out in the presence of an essentially water-immiscible, substantially inert solvent for nickel carbonyl. Instead of a solvent, the nickel carbonyl may be separated from the leach solution by passing a carbon monoxide-containing gas through the leach solution allowing nickel carbonyl to vaporize into the gas and subsequently passing the carbon monoxide-containing into a thermal decomposition zone wherein nickel carbonyl is decomposed to metallic nickel.

The embodiment of the invention is more fully illustrated by the following example.

#### EXAMPLE 36

A nickel sulfide ore containing a pyrrhotite-to-pentalandite ratio of about 5.5 to 1 is crushed, ground and screened to about 85 percent passing 65-mesh screen. The ore is then pumped to flotation cells where a nickel concentrate, a copper concentrate, an iron concentrate and a tailing are separated. The nickel concentrate typically analyzes 5 percent nickel, 1 percent copper, 42 percent iron, 28 percent sulfur and 12 percent moisture.

The concentrate is mixed with siliceous flux and fed into a multi-hearth roaster and heated at exit to about 1,500°F. The calcine formed typically has a sulfur content of about 12.5 percent. The calcine is fed to conveyors which distribute the feed to the reverberatory furnace via fettling pipes. The furnace, operating at a temperature range of 3,000°F. at the burner to 2,400°F. at the flue gas exit, smelts the charge and a matte containing 15 percent nickel-copper is tapped into ladles

- for transfer to converters. The matte with additional siliceous flux is added to the converters and blown with air to produce a low iron, sulfur deficient converter matte having a typical analysis of 47 percent nickel, 30 percent copper, 0.5 percent iron and 22 percent sulfur, the balance being precious metals and impurities.

Converter matte is quenched by pouring into a water spray and then transferred to leach tanks containing aqueous ammoniacal ammonium carbonate. The slurry 10 is then aerated dissolving the nickel, copper and cobalt values and charged to the carbonylation reactor. After sealing the reactor, the charge is pressurized to about 300 psig. with carbon monoxide, heated to about 250°F., and mechanically agitated. After three hours, 15 the reactor is cooled and the remaining carbon monoxide is vented. Nickel carbonyl produced is also vented with the carbon monoxide. Additional carbon monoxide is bubbled through the reaction media to sweep out any remaining nickel carbonyl. The reaction media is 20 decanted and metallic copper is recovered from the reaction vessel. The cobalt is precipitated from the reaction media by injecting oxygen into the reaction media and oxidizing cobalt tetracarbonyl anion to hydrated cobalt oxide which is insoluble in the reaction media. 25 The cobalt oxide is filtered and the filter cake heated to drive off the waters of hydration, producing cobalt oxide for market. The nickel carbonyl is passed through a thermal decomposition zone at about 400°F. and metallic nickel is formed. All of the metals, nickel, 30 copper and cobalt are obtained in good yield.

The carbonylation step of the above example may be carried out in the above example in the presence of a cyanide ion catalyst and/or a water-immiscible, substantially inert solvent, as previously described, and 35 nickel, copper and cobalt obtained in good yields.

One skilled in the art will recognize obvious process variations in the above preferred embodiment. For example, the multi-hearth roaster may be replaced by a fluidized bed roaster with suitable pelletizing means 40 employed prior to roasting. Also, blast furnace or electric arc furnace smelting may be employed with suitable modifications of the feed material, in the case of the blast furnace to prevent blowing out the fine particulates in the fuel.

45 Another preferred embodiment of this invention is similar to the above, but omits the converting step which is employed after smelting. Thus, the smelter matte is oxidatively leached and reductively carbonylated to produce nickel carbonyl. Therefore, a preferred embodiment of this invention is a process for recovering nickel from a nickeliferous sulfide ore, said process comprising:

- a. beneficiating the ore to produce a nickel-enriched concentrate;
- b. roasting the concentrate under oxidizing conditions to produce a calcine having reduced sulfur content;
- c. smelting said calcine in the presence of a siliceous flux to produce a nickel-iron matte;
- d. oxidatively leaching the matte with an aqueous ammoniacal ammonium salt solution by injecting an oxygen-containing gas into a slurry of the matte in the aqueous ammoniacal ammonium salt solution thereby dissolving the nickel values of the matte;
- e. contacting the resultant leach solution with a carbon monoxide-containing gas under conditions

- whereby the nickel values are reduced to form nickel carbonyl;
- f. separating the nickel carbonyl from the leach solution; and
- g. decomposing the nickel carbonyl to metallic nickel.

A preferred method of carrying out the contacting of step (e) is to use an essentially water-immiscible, substantially inert solvent for nickel carbonyl whereby the nickel carbonyl produced is concentrated in the solvent. A most preferred solvent is a saturated aliphatic hydrocarbon. A preferred process of the above invention is further characterized by carrying out the contacting of step (e) above in the presence of an amount of cyanide ion sufficient to catalyze the formation of nickel carbonyl. A most preferred amount of cyanide ion catalyst is from 0.01 to 1 moles of cyanide ion per mole of nickel present. The oxidative leach is preferably carried out with an aqueous ammoniacal ammonium, chloride, carbonate, sulfate or mixtures thereof. Also, aqueous ammonium hydroxide may be employed to form the leach solution. A most preferred aqueous ammoniacal ammonium salt solution is aqueous ammoniacal ammonium carbonate. In lieu of the solvent for nickel carbonyl, the separation from the leach solution of step (f) above may be effected by passing a carbon monoxide-containing gas through the leach solution allowing nickel carbonyl to vaporize into the carbon monoxide-containing gas and subsequently passing the carbon monoxide-containing gas into a thermal decomposition zone wherein nickel carbonyl is decomposed to metallic nickel.

One skilled in the art will recognize that copper and cobalt may also be recovered with the nickel content of the ore. Therefore, a preferred process of this invention is useful for recovering nickel, copper and cobalt from an ore by a process comprising:

- a. beneficiating the ore to produce a concentrate of the ore enriched in nickel, copper and cobalt;
- b. roasting the concentrate under oxidizing conditions to produce a calcine having a reduced sulfur content;
- c. smelting the calcine in the presence of a siliceous flux to produce a nickel-copper-cobalt-iron matte;
- d. converting the matte by blowing with air or oxygen-enriched air in the presence of a siliceous flux at a temperature sufficient to maintain at least part of the matte in a molten state;
- e. oxidatively leaching the converted matte with an aqueous ammoniacal ammonium salt solution by injecting an oxygen-containing gas into a slurry of the converted matte, thereby dissolving the nickel, copper and cobalt values;
- f. contacting the resultant leach solution with a carbon monoxide-containing gas under conditions whereby the nickel, copper and cobalt values are reduced to form nickel carbonyl, metallic copper and cobalt tetracarbonyl anion;
- g. separating the nickel carbonyl from the leach solution;
- h. decomposing nickel carbonyl to metallic nickel;
- i. recovering metallic cobalt from the leach solution;
- j. separating the cobalt from the leach solution by injecting an oxygen-containing gas into the leach solution whereby the cobalt tetracarbonyl anion is oxidized to hydrated cobalt oxide; and

- k. heating said hydrated cobalt oxide at a temperature sufficient to drive off the waters of hydration to produce cobalt oxide.

As previously described in the process for recovering nickel, it is a preferred embodiment of this invention to carry out the oxidative leach of step (e) above with an aqueous ammoniacal ammonium, chloride, carbonate, sulfate or mixture thereof. Also, aqueous ammonium hydroxide may be employed for this purpose. A preferred aqueous ammoniacal ammonium salt solution is aqueous ammoniacal ammonium carbonate. The process may be further characterized by carrying out the contacting of step (f) above in the presence of cyanide ion as a catalyst and in the further presence of an essentially water-immiscible, substantially inert solvent for nickel carbonyl. Instead of the solvent, nickel carbonyl can be separated from the leach solution by utilizing a carbon monoxide sweep to vaporize the nickel carbonyl and pass it into a thermal decomposition zone 20 wherein nickel carbonyl is decomposed to metallic nickel.

This process is illustrated by the following example.

#### EXAMPLE 37

25 A sulfide ore is crushed, ground and screened according to common practice to produce a material suitable for beneficiation. The beneficiation procedure is carried out according to known techniques to yield a concentrate of nickel, cobalt and copper sulfide, and a 30 tailing which is sent to impounding ponds. The concentrate with siliceous flux is roasted at 2,000°F. in a fluidized bed roaster and the calcine charged to an electric arc furnace where it is smelted. The matte tapped off is granulated in a water spray launder and then slurried 35 in an aqueous ammoniacal ammonium carbonate solution. Iron remaining in the matte is reacted to hydrated ferric hydroxide. The leach solution containing dissolved nickel, copper and cobalt values is separated in a series of counter-current decantation thickeners from 40 the residue which is washed to recover any soluble nickel, copper and cobalt values remaining. The resultant leach solution is fed to a pressure reactor with the addition of potassium cyanide as a catalyst and the reactor is pressured with synthesis gas at about 600 psig. 45 The leach solution is heated to about 250°F. and mechanically agitated. After 2 hours, the reactor is cooled and vented to a thermal decomposition zone where the nickel carbonyl formed during the reaction is decomposed to metallic nickel. Additional carbon monoxide is passed through the reaction solution to sweep out all 50 of the nickel carbonyl.

The solution is decanted from the reactor and metallic copper formed during the reaction is recovered.

55 The cobalt is precipitated from the solution by oxidizing the cobalt tetracarbonyl anion forming during the reaction with oxygen to form hydrated cobalt oxide. The hydrated cobalt oxide is then heat treated in a rotary kiln to dry and dehydrate the cobalt oxide.

60 Nickel metal, metallic copper and cobalt oxide are recovered in good yield from this process.

Another source for nickel is the by-product streams from iron ore recovery processes. Since iron and nickel are commonly found together, one problem in most nickel recovery processes has been to separate the large amounts of high iron containing pyrrhotite,  $Fe_7S_8$ . This material contains nickel as substitutes for iron in the pyrrhotite and as pentlandite occlusions which are

not removed by the flotation concentration. Further, by removing a pyrrhotite concentrate this material bypasses smelter operations, thus increasing the capacity of the smelter. On treatment as described below the iron is suitable for use by the steel industry and valuable non-ferrous metals are recovered.

One presently employed process for nickel recovery from pyrrhotite concentrates oxidizes the iron sulfide concentrate in fluid bed roasters to a low-sulfur calcine. The calcine is passed through rotary kilns together with a reducing gas, such as a mixture of carbon dioxide and carbon monoxide in a 1.3:1 ratio, to reduce selectively nickel, copper and cobalt. These metal values are leached in ammonia-ammonium carbonate solution. The solution is treated to recover metal values and reagent. The iron oxide in the residue is pelletized and hardened on a sintering machine. Another process subjects the concentrate to a sulfating roast forming water soluble sulfates of the nickel, copper, and cobalt values. The calcine is leached with water and the solution treated for recovery of metal values. The iron oxide residue is sold as such.

In each case above, a preferred embodiment of this invention is the reductive carbonylation, that is, treating with a carbon monoxide-containing gas, of the ammonia-ammonium carbonate solution or the water soluble metal sulfate solution, respectively, to produce nickel carbonyl, separating the nickel carbonyl and decomposing it to metallic nickel. Copper and cobalt are preferably obtained as metallic copper and as the cobalt tetracarbonyl anion, respectively.

Thus, another preferred embodiment of this invention is a process for the recovery of nickel from a pyrrhotite concentrate, said process comprising:

- a. roasting the concentrate with an oxygen-containing gas whereby a substantially sulfur-free calcine is formed;
- b. heating said calcine with a reducing gas whereby the nickel values are selectively reduced to nickel metal;
- c. oxidatively leaching the reduced calcine with an aqueous ammoniacal ammonium salt solution whereby the nickel is dissolved forming a leach solution;
- d. contacting said leach solution with a carbon monoxide-containing gas under conditions whereby the nickel values are reduced to form nickel carbonyl;
- e. separating said nickel carbonyl from the leach solution; and
- f. decomposing said nickel carbonyl to metallic nickel.

The above process may be further characterized by carrying of the contacting of step (d) in the presence of a catalyst for the formation of nickel carbonyl, such as cyanide ion. A preferred amount of cyanide is from 0.01 to about 1 moles of cyanide ion per mole of nickel.

The contacting of step (d) may also be carried out in the presence of an essentially water-immiscible, substantially inert solvent for nickel carbonyl whereby the nickel carbonyl formed is concentrated in the solvent. A preferred solvent is a saturated aliphatic hydrocarbon as previously described.

Instead of using the inert solvent, nickel carbonyl may preferably be separated from the leach solution according to step (e) by passing a carbon monoxide-containing gas through the leach solution allowing the

nickel carbonyl to vaporize into the carbon monoxide-containing gas and thermally decomposing the nickel carbonyl to metallic nickel.

Cobalt and copper may also be recovered from pyrrhotite in the above process. Thus, a preferred embodiment of this invention is the recovery of nickel, copper and cobalt from a pyrrhotite concentrate by a process comprising:

- a. roasting the concentrate with an oxygen-containing gas whereby a substantially sulfur-free calcine is formed;
- b. heating said calcine with a reducing gas whereby the nickel, copper, and cobalt values are selectively reduced to the metals;
- c. oxidatively leaching the reduced calcine with an aqueous ammoniacal ammonium salt solution whereby the nickel, copper, and cobalt are dissolved forming a leach solution;
- d. contacting said leach solution with a carbon monoxide-containing gas under conditions whereby the nickel, copper, and cobalt values are reduced to form nickel carbonyl, metallic copper, and cobalt tetracarbonyl anion;
- e. separating said nickel carbonyl from the leach solution;
- f. decomposing said nickel carbonyl to metallic nickel;
- g. recovering said metallic copper;
- h. separating said cobalt from the leach solution by injecting an oxygen-containing gas into the leach solution oxidizing said cobalt tetracarbonyl anion to hydrated cobalt oxide; and
- i. heating said hydrated cobalt oxide to drive off the waters of hydration to produce cobalt oxide.

The previously described use of cyanide catalyst and water-immiscible, inert solvent of carbon monoxide-containing gas sweep as previously described are applicable to this process and are preferred embodiments thereof. This process will be more fully illustrated by the following example.

#### EXAMPLE 38

A pyrrhotite concentrate is employed having a typical analysis as follows:

0.75% nickel  
0.05% copper  
58% iron  
35% sulfur  
2% silica

The concentrate is prepared by standard flotation techniques from a nickel sulfide ore and averages 90 percent minus 200-mesh. The pyrrhotite feed is charged to a fluidized bed roaster which is operated at 1,400°F. and burned with preheated air. The calcine discharging from the roaster contains about 0.2 percent sulfur. The calcine is fed to a concurrently natural gas-fired rotary kiln heated to 1,600°F. at the charge end and 1,300°F. at the discharge exit. A gaseous reducing atmosphere results from the combination having a CO<sub>2</sub>/CO ratio of 1.3 at the charge end and 1.6 at the discharge end. The metal oxides produced in the roaster are reduced to leachable forms of the metals in the rotary kiln with only a small portion of the nickel and iron remaining as the sulfide. From the main portion of the rotary kiln the reduced ore moves into air cooled tubes and then discharges into quench tanks. The pulp from the quench tank is leached with aqueous ammoniacal ammonium

carbonate in agitated aeration tanks to extract the nickel, copper, and cobalt. The aeration is carried out at 130°F. under atmospheric pressure. The pregnant solution of nickel, copper, and cobalt is separated from the ferric hydroxide produced and charged to a pressure reactor for carbonylation. Potassium cyanide is added to the reactor as a catalyst and the reactor is pressurized to about 300 psig. with carbon monoxide. The leach solution is heated to about 250°F. and agitated mechanically. After 2 hours the reactor is cooled and vented to a thermal decomposition zone where nickel carbonyl formed during the reaction is decomposed to metallic nickel. Additional carbon monoxide is passed through the reaction solution to sweep out all of the nickel carbonyl.

The copper deposits on the bottom of the reaction vessel and is removed as such. The cobalt is separated from the solution by injecting air into it, producing insoluble hydrated cobalt oxide. The hydrated cobalt oxide is then filtered from the solution and heated to drive off the water of hydration.

The nickel, copper, and cobalt are recovered in good yield. The iron oxide is produced from ferric hydroxide by sintering on a traveling grate machine and is also recovered in good yield for marketing to steel producers.

The above example may be repeated with similar results using HCN gas as a catalyst, or synthesis gas as the carbonylating gas. Another process expedient which can be used to advantage is to heat the pregnant leach liquor to drive off ammonia values and precipitate the nickel and cobalt as basic carbonates. These can then be mixed with more ammonia to concentrate the metal values, decrease the volume of material which must be processed, and allow any adjustment required in the solution to be made prior to carbonylating.

Nickel recovery from pyrrhotite concentrate via a sulfating roast is carried out in a similar manner, except that sodium sulfate is added to the roaster and the calcine consists of iron oxide and the sulfates of nickel, copper, and cobalt. These are extracted in a water leach and can be carbonylated in accordance with the above teachings.

Another preferred embodiment of the process of this invention is the recovery of nickel from scrap metal. In this process, schematically represented in FIG. 9, the scrap metal is comminuted to a size desirable for further processing. While the size is not critical, a proportionately large surface for subsequent action is presented when the scrap is less than about 100 mesh. After size reduction, the scrap metal is leached with an ammoniacal ammonium salt solution to selectively dissolve nickel and its associated metals. The leach solution is then contacted with a carbon monoxide-containing gas and nickel carbonyl is formed, separated from the reaction solution and nickel metal is recovered. Copper and cobalt present in the leach solution also react and may be recovered after separation from the reaction mixture in the manner previously described.

Therefore, a further preferred embodiment of this invention is a process for recovery of nickel values from scrap metal containing a recoverable amount of nickel, said process comprising:

- a. comminuting said scrap metal;
- b. oxidatively leaching the comminuted scrap metal with an aqueous ammoniacal ammonium salt solution by injecting an oxygen-containing gas into a

slurry of said comminuted scrap metal in said aqueous ammoniacal ammonium salt solution, thereby dissolving the nickel values of said scrap metal;

- c. contacting the resultant leach solution with a carbon monoxide-containing gas under conditions whereby the nickel values are reduced to nickel carbonyl;
- d. separating said nickel carbonyl from said leach solution; and
- e. decomposing said nickel carbonyl to metallic nickel.

As previously described, the contacting of step (c) can preferably be carried out in the presence of an essentially waterimmiscible, substantially inert solvent for nickel carbonyl whereby the nickel carbonyl produced is concentrated in the solvent. A preferred solvent is a saturated hydrocarbon.

The above process may be further characterized by carrying out the contacting of step (c) in the presence of an amount of cyanide sufficient to catalyze the formation of nickel carbonyl. A preferred amount of cyanide ion is from 0.01 to 1 mole of cyanide ion per mole of nickel present.

The aqueous ammoniacal ammonium salt is preferably selected from aqueous ammoniacal ammonium chloride, carbonate, sulfate, or mixtures thereof. Also, aqueous ammonium hydroxide may be employed. A most preferred aqueous ammoniacal ammonium salt solution is aqueous ammoniacal ammonium carbonate.

Instead of using the inert solvent, nickel carbonyl may be separated from the leach solution after carbonylation by passing a carbon monoxide-containing gas through the leach solution allowing the nickel carbonyl to vaporize into the carbon monoxide-containing gas and then passing the gas into a thermal decomposition zone wherein the nickel carbonyl is thermally decomposed to metallic nickel.

When the scrap metal contains recoverable amounts of copper and cobalt in addition to nickel, a preferred embodiment of this invention is a process for recovering nickel, copper, and cobalt, said process comprising:

- a. comminuting the scrap metal;
- b. oxidatively leaching the comminuted scrap metal with an aqueous ammoniacal ammonium salt solution by injecting an oxygen-containing gas into a slurry of said comminuted scrap metal in said aqueous ammoniacal ammonium salt solution, thereby dissolving the nickel, copper and cobalt values of said scrap metal;
- c. contacting the resultant leach solution with a carbon monoxide-containing gas under conditions whereby the nickel, copper, and cobalt values are reduced to form nickel carbonyl, metallic copper, and cobalt tetracarbonyl anion;
- d. separating said nickel carbonyl from said leach solution;
- e. decomposing said nickel carbonyl to metallic nickel;
- f. recovering said metallic copper from said leach solution;
- g. separating said cobalt from the leach solution by injecting an oxygen-containing gas into said leach solution whereby said cobalt tetracarbonyl anion is oxidized to hydrated cobalt oxide; and
- h. heating said hydrated cobalt oxide at a temperature sufficient to drive off the waters of hydration to produce cobalt oxide.

From the previously described processes it is apparent that this process may employ an aqueous ammoniacal ammonium salt solution selected from aqueous ammoniacal ammonium chloride, carbonate, sulfate, or mixtures thereof; also, aqueous ammonium hydroxide may be employed. The process may also be characterized further by the use of a promoter such as an amount of cyanide ion sufficient to catalyze the formation of nickel carbonyl. It may also use an inert solvent for nickel carbonyl in the carbonylation step, as previously described. Instead of the solvent, a carbon monoxide-containing gas may be employed to sweep out the nickel carbonyl into a thermal decomposition zone, also as previously described.

Scrap metal suitable for use in this preferred embodiment may be crushed auto bodies; iron, steel, nickel, copper, and other metal machinings, turnings, or filings; used electric cable and wire; and the like. Thus, the source of scrap is not critical, so long as recoverable amounts of nickel, copper, and cobalt are contained therein.

One source of nickel which contains vast amounts of recoverable nickel and which has been heretofore largely ignored because of its inaccessibility is the ocean floor. Estimates of nickel available from this source are  $3.2 \times 10^9$  metric tons of nickel, or about 220 times the world reserves based on 1958 statistics available. The most practical and economically feasible source of nickel from the ocean is black, hydrous manganese-dioxide concretions on the floors of the ocean. These manganese sea nodules contain from 2.0 - 0.31 percent nickel, 2.3 - 0.6 percent cobalt, and 1.6 - 0.28 percent copper. The average composition of manganese nodules in the Pacific Ocean is 0.99 percent nickel, 0.35 percent cobalt, and 0.53 percent copper.

Manganese sea nodules are found in a variety of shapes and sizes. The largest nodule ever recorded was over 18,000 pounds. However, manganese sea nodules generally average from 0.8 - 1.5 inches in diameter and usually do not exceed about 3 inches.

Estimates of the concentrations of manganese sea nodules have been made from photographs and dredging samples of the sea floor. One estimate sets the total tonnage of nodules in the Pacific Ocean at 1,656 billions of metric tons, with over half of this amount about 900 billions of metric tons being located in the central region of the Pacific. In this region it is estimated, based on a limited sampling, that about 0.4 - 7.6 pounds of nodules per square foot exist. Estimates in other portions of the Pacific range from 0.1 - 4.6 pounds per square foot of nodules. However, no intensive sampling has been done to prove out a given location.

The manganese sea nodules may be recovered by dredging with bucket-ladder, wire-line, and hydraulic dredges. For example, drag-bucket, clamshell-dredges, and air-lift hydraulic dredges have been used and are well known to skilled practitioners of the dredging art. Other methods have been proposed for recovery of sea-floor minerals at depths over 1,000 feet, including unmanned crawler-type units, manned bathyscaphes of both the crawler-type and submarines. However, only the well-known deep-sea drag-dredge is practical for commercial operations in the near future.

Processing manganese sea nodules is much like other sources of nickel. Therefore, manganese sea nodules are amenable to the process of this invention. Thus, a preferred embodiment of this invention is a process for re-

covering nickel values from manganese nodules, said process comprising:

- a. comminuting said nodules;
- b. subjecting the comminuted nodules to a reducing roast to convert the nickel values to nickel metal;
- c. cooling the reduced nodules under non-oxidizing conditions;
- d. oxidatively leaching said reduced nodules with an aqueous ammoniacal ammonium carbonate solution by injecting an oxygen-containing gas into a slurry of said reduced nodules in said aqueous ammoniacal ammonium carbonate solution;
- e. contacting the resultant leach solution containing nickel ammine salt complexes with a carbon monoxide-containing gas under conditions whereby the nickel values are reduced to form nickel carbonyl;
- f. separating said nickel carbonyl from the leach solution; and
- g. decomposing said nickel carbonyl to metallic nickel.

As previously described in the foregoing preferred embodiments, the above process can be further characterized by carrying out the contacting of step (c) in the presence of an essentially water-immiscible, substantially inert solvent for nickel carbonyl whereby the nickel carbonyl is concentrated in said solvent. A preferred solvent is a saturated hydrocarbon. Also, a preferred process of this embodiment is further characterized by carrying out the contacting of said step (c) in the presence of an amount of cyanide ion sufficient to catalyze the formation of nickel carbonyl. A preferred amount of cyanide ion is from 0.01 to 1 mole of cyanide ion per mole of nickel.

The aqueous ammoniacal ammonium salt solution is preferably selected from aqueous ammoniacal ammonium chloride, carbonate, sulfate or mixtures thereof. Also, aqueous ammonium hydroxide may be used. A preferred aqueous ammoniacal ammonium salt is aqueous ammoniacal ammonium carbonate.

Instead of carrying out the contacting in a solvent and separating the nickel carbonyl thereby, nickel carbonyl produced is preferably separated from the leach solution by passing a carbon monoxide-containing gas through the leach solution allowing the nickel carbonyl to vaporize into the carbon monoxide-containing gas and subsequently passing said carbon monoxide-containing gas into a thermal decomposition zone wherein nickel carbonyl is thermally decomposed to metallic nickel.

From the above preferred embodiment and the foregoing descriptions of other preferred embodiments it should be clear that this process also may be employed to recover nickel, copper, and cobalt from manganese nodules. Such a preferred embodiment is a process for recovering nickel, copper, and cobalt from manganese nodules by a process comprising:

- a. comminuting said manganese nodules;
- b. subjecting the comminuted nodules to a reducing roast to convert the nickel, copper and cobalt to nickel metal, copper metal, and cobalt metal;
- c. cooling the reduced nodules under non-oxidizing conditions;
- d. oxidatively leaching said reduced nodules with an aqueous ammoniacal ammonium carbonate solution by injecting an oxygen-containing gas into a

- slurry of said reduced nodules in said aqueous ammoniacal ammonium carbonate solution;
- e. contacting the resultant leach solution containing nickel, copper, and cobalt ammine salt complexes with a carbon monoxide-containing gas under conditions whereby the nickel, copper, and cobalt values are reduced to nickel carbonyl, metallic copper and cobalt tetracarbonyl anion;
- f. separating said nickel carbonyl from said leach solution;
- g. decomposing said nickel carbonyl to metallic nickel;
- h. recovering said metallic copper;
- i. separating the cobalt from the leach solution by injecting an oxygen-containing gas into said solution whereby said cobalt tetracarbonyl anion is oxidized to hydrated cobalt oxide; and
- j. heating said hydrated cobalt oxide at a temperature sufficient to drive off the waters of hydration to produce cobalt oxide.

Of course, the previously described process expedites of using a solvent and an amount of cyanide ion sufficient to catalyze the formation of nickel carbonyl are also preferred embodiments of this process. Instead of the solvent, a carbon monoxide-containing gas may be used to sweep out the nickel carbonyl to the thermal decomposition zone.

In either of the foregoing embodiments using manganese nodules, the comminuted nodules may be subjected to a reducing roast prior to the leach step to convert a substantial amount of the nickel, copper, or cobalt to the metal. Also, instead of using an ammoniacal ammonium salt leach the nodules may be leached with acid (e.g., concentrated  $H_2SO_4$ ) to dissolve the nickel, copper, and cobalt values. The free acid can then be neutralized using for example coral mud or clamshells and the neutralized leach rendered basic with ammonia. This solution can then be subjected to the reductive carbonylation and subsequent steps described above and throughout this specification.

In all of the preferred embodiments described hereinabove, the conditions of catalyst, aqueous ammoniacal ammonium salt, solvent, temperature, pressure, carbon monoxide-containing gas, oxygen-containing gas, and carbon monoxide sweep are similar to those described broadly for the general process of reductive carbonylation and are applicable to the specific processes wherein this step is employed.

Therefore, it is desired that the invention be limited only within the lawful scope of the appended claims.

We claim:

1. A process for the recovery of nickel from an aqueous solution or slurry of a soluble nickel salt, said aqueous solution or slurry additionally containing a soluble copper salt or cobalt salt, or both, said process comprising contacting said aqueous solution or slurry with a carbon monoxide-containing gas under conditions of temperature and pressure sufficient to reduce said soluble nickel salt to nickel carbonyl, separating said nickel carbonyl from the treated solution or slurry containing metallic copper or cobalt values, or both, and decomposing said nickel carbonyl to metallic nickel.

2. A process of claim 1 wherein said solution or slurry is an ammonium salt solution or slurry.

3. A process of claim 2 wherein said ammonium salt solution or slurry is an ammoniacal ammonium salt solution or slurry.

4. A process of claim 3 wherein said ammoniacal ammonium salt solution is selected from the group consisting of ammoniacal ammonium chloride, carbonate, sulfate, and mixtures thereof.
5. A process of claim 4 wherein said ammoniacal ammonium salt solution or slurry is an ammoniacal ammonium carbonate solution or slurry.
6. A process of claim 5 wherein the molar ratio of ammonia to metal in said ammoniacal ammonium carbonate solution is from 0:1 to about 100:1.
7. A process of claim 6 wherein the molar ratio of ammonia to metal in said ammoniacal ammonium carbonate solution is from 0:1 to 10:1.
8. A process of claim 6 wherein said reaction is carried out at a pressure of from 50 to about 3,000 psig. and a temperature of from about 50° to about 250°C.
9. A process of claim 8 wherein said temperature is from 100° to about 175°C.
10. A process of claim 1 wherein said reaction is carried out in the presence of a catalytic amount of a ligand selected from the group consisting of cyanide, sulfide, cysteine, and tartrate.
11. A process of claim 10 wherein said reaction is carried out at a temperature of from 50° to about 250°C. and a pressure of from 50 to about 1,800 psig.
12. A process of claim 10 wherein said ligand is present at a ratio of from 0.01 to 1 mole of said ligand per mole of said nickel.
13. A process of claim 12 wherein said ligand is present at a ratio of from 0.01 to 0.5 mole of said ligand per mole of said nickel.
14. A process of claim 12 wherein said ligand is cyanide ion.
15. A process of claim 1 wherein said carbon monoxide-containing gas is selected from the group consisting of carbon monoxide and synthesis gas.
16. A process of claim 15 wherein said carbon monoxide-containing gas is carbon monoxide.
17. A process of claim 1 wherein said contacting is carried out in the presence of an essentially water-immiscible, substantially inert solvent for nickel carbonyl whereby said nickel carbonyl is concentrated in said solvent.
18. A process of claim 17 wherein said solvent is a saturated aliphatic hydrocarbon.
19. A process of claim 4 further characterized by carrying out said contacting in the presence of an amount of cyanide ion sufficient to catalyze the formation of said nickel carbonyl.
20. A process of claim 19 wherein said contacting is carried out in the presence of an essentially water-immiscible, substantially inert solvent for nickel carbonyl wherein said nickel carbonyl formed is concentrated in said solvent.
21. A process of claim 1 wherein said nickel carbonyl is separated from said solution by passing a carbon monoxide-containing gas through said solution, allowing said nickel carbonyl to vaporize into said carbon monoxide-containing gas and subsequently passing said carbon monoxide-containing gas into a thermal decomposition zone wherein said nickel carbonyl in said carbon monoxide-containing gas is decomposed to metallic nickel.
22. A process of claim 1 wherein said solution or slurry is aqueous ammonium hydroxide.
23. A process for the manufacture of nickel said process comprising
- a. establishing an aqueous solution or slurry contain-

- ing nickel derived from a source of nickel ore,  
b. contacting said solution or slurry with a carbon monoxide-containing gas under conditions of temperature and pressure sufficient to form nickel carbonyl,  
c. separating said nickel carbonyl from said solution or slurry, and  
d. decomposing said nickel carbonyl to obtain metal-

lic nickel.

24. A process of claim 1 wherein said aqueous solution or slurry contains an ammonium salt or ammonium hydroxide and a catalytic amount of cyanide ion and  
5 the reaction is carried out at a temperature of from about 50° to about 250 °C and a pressure of from about 50 to about 3,000 psig.

\* \* \* \* \*

10

15

20

25

30

35

40

45

50

55

60

65

UNITED STATES PATENT OFFICE  
CERTIFICATE OF CORRECTION

Patent No. 3,775,099 Dated November 27, 1973

Inventor(s) Thomas H. Coffield and Kestutis A. Keblyns

It is certified that error appears in the above-identified patent and that said Letters Patent are hereby corrected as shown below:

Col. 8, line 38, reads "rane", should read -- range --.  
Col. 13, line 24, reads under Example 8 "101", should read -- 110 --. Col. 13, first line of footnote 1, reads "NiSO<sub>3</sub>", should read -- NiSO<sub>4</sub> --. Col. 13, line 63, reads "neckel", should read -- nickel --. Col. 14, line 49, reads "THus", should read -- Thus --. Col. 15, line 17, reads "neckel", should read -- nickel --. Col. 15, line 44, reads "saturated", should read -- saturated --. Col. 15, line 67, reads "Rathre", should read -- Rather --. Cancel columns 17 thru 60 of the printed patent and substitute the attached columns 17 thru 20.

Signed and sealed this 30th day of April 1974.

(SEAL)

Attest:

EDWARD M.FLETCHER, JR.  
Attesting Officer

C. MARSHALL DANN  
Commissioner of Patents